# EUROPEAN PATENT SPECIFICATION

(11) **EP 3 158 095 B1**
(45) Date of publication and mention of the grant of the patent: **02.05.2018**
(21) Application number: 08864853.0
(22) Date of filing: 19.12.2008
(51) Int. Cl.: C22C 9/06, C22C 9/10, C22F 1/08

(54) **COPPER-NICKEL-SILICON ALLOYS**
KUPFER-NICKEL-SILIZIUM-LEGIERUNGEN
ALLIAGES DE CUIVRE-NICKEL-SILICIUM

(30) Priority: 21.12.2007 US 16441; 14.04.2008 US 44900; 17.12.2008 US 336731
(43) Date of publication of application: 26.04.2017
(73) Proprietor: GBC Metals, LLC, East Alton IL 63024 (US); Wieland-Werke AG, 89079 Ulm (DE)
(72) Inventor: MUTSCHLER, Ralph, A., Edwardsville IL 62025 (US); ROBINSON, Peter, William, Glen Carbon IL 62034 (US); TYLER, Derek, E., Cheshire CT 06410 (US); KAUFLER, Andrea, D-89079 Ulm (DE); KUHN, Hans, Achim, D-89079 Ulm (DE); HOFMANN, Uwe, D-89079 Ulm (DE)
(74) Representative: Dziewior, Joachim
(86) International application number: PCT/US2008/087705
(87) International publication number: WO 2009/082695

(56) References cited:
- US-A- 4 594 221
- US-A- 4 728 372
- US-A1- 2004 079 456
- US-A1- 2006 196 586
- US-A1- 2007 131 315

## Description

### CROSS-REFERENCE TO RELATED APPLICATIONS

### BACKGROUND

This invention relates to copper base alloys, and in particular to copper-nickel-silicon base alloys.

Copper-nickel-silicon base alloys are widely used for the production of high strength, electrically conductive parts such as connectors and lead frames. C7025, developed by Olin Corporation, is an important example of a copper-nickel-silicon base alloy that provides good mechanical (yield strength 95 ksi - 110 ksi / 655 MPa - 758 MPa) and good electrical properties (35% IACS). See U.S.Patent Nos. 4,594,221 and 4,728,372, incorporated herein by reference. More recently, C7035, a cobalt modified copper, nickel, silicon alloy, has been developed by Olin Corporation and Wieland Werke, which can provide even better mechanical (yield strength 100 ksi - 130 ksi / 689 MPa - 896 MPa) and electrical properties(40-55% IACS). See U.S. Patent No. 7,182,823, incorporated herein by reference.

The properties of copper alloys that can be important include formability, conductivity, strength, ductility, and resistance to stress relaxation.

Formability is typically evaluated by a bend test where copper strips are bent 90°around a mandrel of known radiu s. A roller bend test employs a roller to form the strip around the mandrel. Alternatively, a v-block test uses the mandrel to push the strip into an open die, forcing it to conform to the radius of the mandrel. For both tests the minimum bend radius (mbr) as a function of strip thickness (t) is then reported as mbr/t. The minimum bend radius is the smallest radius mandrel around which a strip can be bent without cracks visible at a magnification of 10x to 2Ox. Generally mbr/t is reported for both good way bends, defined as the bend axis is normal to the rolling direction, and for bad way bends, defined as the bend axis is parallel to the rolling direction. An mbr/t of up to 4 t for both good way bends and bad way bends is deemed to constitute good formabiüty. More preferred is an mbr/t of up to 2.

Electrical conductivity is typically measured as a percentage of IACS. IACS refers to International Annealed Copper Standard that assigns "pure" copper a conductivity value of 100% IACS at 20°C T hroughout this disclosure, all electrical and mechanical testing is performed at room temperature, nominally 20° C, unless otherwise specified. The qualifying expression "about" indicates that exactitude is not required and should be interpreted as +/-10% of a recited value.

Strength is usually measured as yield strength. A high strength copper alloy has a yield strength in excess of 95 ksi (655,1 MPa) and preferably in excess of 110 ksi (758,5 MPa). As the gauge of the copper alloy formed into components decreases and as miniaturization of these components continues, a combination of strength and conductivity for a given temper will be more important than either strength or conductivity viewed alone.

Ductility can be measured by elongation. One measure of elongation is A10 elongation, which is the permanent extension of the gauge length after fracture, expressed as a percentage of the original gauge length Lo where Lo is taken equal to 10 mm.

Acceptable resistance to stress relaxation is viewed as at least 70% of an imparted stress remaining after a test sample is exposed to a temperature of 150°C for 3000 hours and at least 90% of an imparted stress remaining after a test sample is exposed to a temperature of 105°C for 1000 hours.

Stress relaxation resistance was measured via the ring method [Fox A.: Research and Standards 4 (1964) 480] wherein a strip of 50 mm length is clamped onto the outer radius of a steel ring initiating stress at the outer surface of the strip. With exposure to elevated temperatures elastic stresses change into plastic deformation. This process depends upon time, temperature and initial stress defined by the radius of the steel ring. Experiments were performed between 50°C/96 h and 210°C/384 h. After each annealing the remaining flexion of the strip is measured and the corresponding stress reduction calculated according to [Graves G.B.: Wire Industry 46 (1979) 421]. Using the Larson-Miller-Parameter P an extrapolation from the performed short time experiments at higher temperatures to long time experiments at lower temperatures can be done [Boegel A.: Metall 48 (1994) 872].

Stress relaxation may also be measured by a lift-off method as described in ASTM (American Society for Testing and Materials) Standard E328-86. This test measures the reduction in stress in a copper alloy sample held at fixed strain for times up to 3000 hours. The technique consists of constraining the free end of a cantilever beam to a fixed deflection and measuring the load exerted by the beam on the constraint as a function of time at temperature. This is accomplished by securing the cantilever beam test sample in a specially designed test rack. The standard test condition is to load the cantilever beam to 80% of the room temperature 0.2% offset yield strength. If the calculated deflection exceeds about 0.2 inch (5 mm), the initial stress is reduced until the deflection is less than 0.2 inch (5 mm) and the load is recalculated. The test procedure is to load the cantilever beam to the calculated load value, adjust a threaded screw in the test rack to maintain the deflection, and locking the threaded screw in place with a nut. The toad required to lift the cantilever beam from the threaded screw is the initial load. The test rack is placed in a furnace set to a desired test temperature. The test rack is periodically removed, allowed to cool to room temperature, and the load required to lift the cantilever beam from the threaded screw is measured. The percent stress remaining at the selected log times is calculated and the data are plotted on semi-log graph paper with stress remaining on the ordinate (vertical) and log time on the abscissa (horizontal). A straight line is fitted through the data using a linear regression technique. Interpolation and extrapolation are used to produce stress remaining values at 1, 1000, 3000, and 100,000 hours.

The resistance to stress relaxation is orientation sensitive and may be reported in the longitudinal (L) direction where 0°testing is conducted with the long dimension of the test sample in the direction of strip rolling and the deflection of the test sample is parallel to the strip rolling direction. The resistance to stress relaxation may be reported in the transverse (T) direction where 90° testing is conducted with the long dimension of the test sample perpendicular to the strip rolling direction and the deflection of the test sample is perpendicular to the strip rolling direction.

Table 1 shows the mechanical and electrical properties of some of the commercially available copper alloys of which the inventors are aware:

| **Table 1 Examples of properties of currently available Be-free Cu-based alloys** | | | | |
|---|---|---|---|---|
| Alloy | Company | Composition | El. Conductivity (%IACS) | Yield Strength, ksi |
| C7025 | Olin Brass | Cu+3.0Ni+0.60Si+0.15Mg | >35 | 95-110 |
| EFTEC-75 | Furukawa | Cu+3.2Ni+0.65Si+0.5Zn+0.50Sn | 25 | 116 |
| EFTEC-23Z | Furukawa | Cu+2.5Ni+0.6Si+0.5Zn+0.03Ag | 53 | 101-116 |
| EFTEC-97 | Furukawa | Cu+2.3Ni+0.65Si+0.5Zn+0.15Sn+0.1Mg | 40 | 110 |
| EFTEC-98 | Furukawa | Unknown | 38 | 104-136 |
| EFTEC-98S | Furukawa | Cu+3.8Ni+0.93Si+0.48Zn+0.18Sn+0.13Mg+0.3Cr | 38 | 95-129 |
| K62 | Wieland | Cu+0.3Cf+0.4NM.6Sn+0.03Tt | 52 | 100 |
| KLF-125 | Kobe Steel | Cu+3.2Ni+0.70Si+0.3Zn+1.25Mn | 35 | 100 |
| CAC-65 | Kobe Steel | Cu+3.2Ni+0.70Si+1.0Zn+0.50Sn | 46 | 94 |
| MAX 251 | Mitsubishi Shindo | Cu+2.0Ni+0.50Si+0.50Sn | 45 | 89 |
| Max375 | Mitsubishi | Cu+2.85Ni+0.7Si+0.5Zn+0.5Sn+0.015Mg | 42 | 91-116 |
| KLF-1 | Kobe Steel | Cu+3.2Ni+0.70Si+0.3Zn+0.50Mn | 55 | 88 |
| C7027 | Olin Brass | Cu+2.0Ni+0.60Si+0.60Zn+0.50Sn | >40 | >80 |
| C18080/K88 | Olin/Wieland | Cu+0.5Cr+0.1Ag+0.08Fe+0.06Ti+0.03Si | 80 | 80 |
| C18070/K75 | Wieland | Cu+0.2Cr+0.1Ti+0.02Si | >75 | 70 |
| PMC 102 | Poongsan | Cu+1.3Ni+0.25Si+0.05P | 60 | 75 |
| C7035/K57 | Olin/Wieland | Cu+1.4Ni+1.1Co+0.6Si | >45 | 110-130 |
| NKC388 | Nippon Minigg | Cu+3.8Ni+0.85Si+0.18Mg-0.1Mn | 35-45 | 112-125 |
| HCL 305 | Hitachi | Cu+2.5M+0.5Si+1.7Zn+0.02P | 42 | 87-102 |
| HCL 307 | Hitachi | Cu+3.0Ni+0.7Sn-1.7Zn+0.3Sn+0.02P | 35 | 102-112 |

As good as these alloys are, and as widespread their use, there remain applications where alloys with higher strength and in particular higher strength without sacrificing other desirable properties such as conductivity, resistance to stress relaxation, and/or formability. While beryllium coppers can provide high strength, because of their beryllium content, they are not suitable for many applications. Among beryllium-free copper alloys, high strength (e.g., yield strength above about 130 ksi / 896 MPa) is usually accompanied by significant diminishment of other desirable properties, in particular formability. US 2007/0079 456 discloses a copper alloy with 1-2.5 wt.% Nickel.

### SUMMARY

The copper based alloy and a method of making the copper based alloy according to the invention are given in the claims. One aspect of the present invention is an age-hardening copper-nickel-silicon base alloy that can be processed to make a commercially useful strip product for use in electrical connectors and interconnections for the automotive and multimedia industries, in particular, and for any other applications requiring high yield strength and moderately high electrical conductivity in a strip, plate, wire or casting. Another aspect of the present invention is a processing method to make a commercially useful strip product for use in electrical connectors and interconnections for the automotive and multimedia industries and any other applications requiring high yield strength and moderately high electrical conductivity.

Preferred embodiments are given in claims 2 and 4. This alloy is processed to have a yield strength of at least about 140 ksi (965 MPa), and an electrical conductivity of at least about 30% IACS.

The alloys are preferably processed to have a yield strength of at least about 143 ksi (986 MPa), and an electrical conductivity of at least about 37% IACS.

The ratio of (Ni+Co)/(Si-Cr/5) is preferably between about 3.5 and about 5.0. The Ratio of Ni/Co is preferably between about 3 and about 5.

The alloys and processing methods of the various embodiments provide copper base alloys having an improved combination of yield strength and electrical conductivity, and preferably stress relaxation resistance as well. In particular the alloys have higher strength and greater resistance to stress relaxation than previously achieved with Cu-Ni-Si alloys, while maintaining reasonable levels of conductivity.

### BRIEF DESCRIPTION OF THE DRAWINGS

Fig. 1 is a flow chart of the treatment of the alloys in Example 1 ;
Fig. 2 is a flow chart of the treatment of the alloys in Example 2;
Fig. 3 is a flow chart of the treatment of the alloys in Example 3;
Fig. 4 is a graph of the yield strength versus conductivity for the alloys of Example 3;
Fig. 5 is a graph of yield strength versus bend formability (MBR/t) for the alloys of Example 3;
Fig. 6 is a flow chart of the treatment of the alloys of Example 4;
Fig. 7 is a graph of yield strength versus conductivity for the alloys of Table 5 processed by a SA-CR-age-CR-age process of Example 4;
Fig. 8 is a graph of yield strength versus bend formability (MBR/t) for the alloys of Table 5 processed by SA-CR-age-CR-age process of Example 4;
Fig. 9 is flow chart of the treatment of the alloys in Example 5;
Fig. 10 is a graph of yield strength vs Ni/Co ratio for alloys without chromium having similar alloying levels of Example 5;
Fig. 11 is flow chart of the treatment of the alloys in Example 6;
Fig. 12 is a flow chart of the treatment of the alloys in Example 7;
Fig. 13 is a graph showing the effect of stoichiometric ratio on yield strength in copper-nickel-chromium-silicon alloys from Example 7;
Fig. 14 is a graph showing the effect of stoichiometric ratio on yield strength in copper-nickel-cobalt-silicon alloys from Example 7;
Fig. 15 is a graph showing the effect of effect of stoichiometric ratio on yield strength in copper-nickel-chromium-cobalt-silicon alloys from Example 7;
Fig. 16 is a graph showing the effect of stoichiometric ratio on electrical conductivity in copper-nickel-chromium-silicon alloys from Example 7;
Fig. 17 is a graph showing the effect of stoichiometric ratio on electrical conductivity in copper-nickel-cobalt-silicon alloys from Example 7;
Fig. 18 is a graph showing the effect of stoichiometric ratio on electrical conductivity in copper-nickel-chromium-cobalt-silicon alloys from Example 7;
Fig. 19 is a flow chart of the treatment of the alloys in Example 8;
Fig. 20 is a graph showing the effect of stoichiometric ratio on %IACS in Example 8 alloys processed by the SA-CR-age-CR-age approach with 475°C/300°C ages.
Fig. 21 is a graph showing the effect of stoichiometric ratio on yield strength in Example 8 alloys processed by the SA-CR-age-CR-age approach with 475°C/300°C ages;
Fig. 22 is a flow chart of the treatment of the alloys in Example 9
Fig. 23 is a schematic diagram of tapered edge hot rolling specimen;
Fig. 24 is a photograph of hot rolled K224 (without Cr), showing large edge cracks;
Fig. 25 is a photograph of hot rolled K225 (0.11 Cr), showing no edge cracks;
Fig. 26A is photograph of the results from tool wear testing of non-Cr alloy RN033407; and
Fig. 26B is a photograph of the Result from tool wear test of Cr containing alloy RN834062;
Fig. 27 is a flow chart of the treatment of the alloys in Example 10;
Fig. 28 is a graph showing the effect of stoichiometric ratio on %IACS in Example 8 and Example 10 (low Cr and Mn) alloys processed by the SA-CR-age-CR-age approach with 475°C/300°C ages; and
Fig. 29 is a graph showing the effect of stoichiometric ratio on yield strength in Example 8 and Example 10 (low Cr and Mn) alloys processed by the SA-CR-age-CR-age approach with 475°C/300°C ages;
Fig. 30 is a flow chart of the treatment of the alloys in Example 11 ; and
Fig. 31 is a flow chart of the treatment of the alloys in Example 12;
Fig. 32 is a flow chart of the treatment of the alloys in Example 13;
Fig. 33 is a flow chart of the treatment of the alloys in Example 14;
Fig. 34 is a flow chart of the treatment of the alloys in Example 15;
Fig. 35 is a flow chart of the treatment of the alloys in Example 16;
Fig. 36 is a graph of 90°V-block - MBR/t BW versus yield strength for alloys and processes of Examples 13, 14, 15, and 16; and
Fig. 37 is a graph of %IACS versus yield strength for alloys and processes of Examples 13,14,15, and 16.

### DETAILED DESCRIPTION

There is a need in the marketplace for copper strip alloys with higher strength and electrical conductivity, along with good stress relaxation resistance. This combination of properties is particularly important for parts that are formed into various electrical interconnections for use in multimedia electrical connector and terminal applications. Commercially available copper alloys, such as C510 (phosphor bronze), C7025, C7035, C17410 and C17460 are being used in these applications for their generally favorable combinations of strength and conductivity. However, while these alloys have adequate strength for most current carrying applications, the continuing trend for miniaturization of components demands copper alloys that offer high strength in combination with reasonably good electrical conductivity and reasonably good stress relaxation resistance along with reasonable cost. It is also desirable to minimize or eliminate potentially toxic alloying elements such as beryllium.

Alloys that are used for multimedia interconnects require high strength to avoid damage during connector insertion and to maintain good contact force while in service. For these applications, good but not especially high electrical conductivity is all that is required, since the conductivity merely needs to be enough to carry a signal current, and need not be the high levels needed to avoid excessive l²R heating in higher power applications. For these applications, there are even more stringent requirements for mechanical stability at room and slightly elevated service temperatures, as characterized by good stress relaxation resistance at about 100°C, for example.

The alloy compositions of the preferred embodiments of this invention, and the scheme used to process to the finish tempers surprisingly provide highly desirable combination of properties for meeting the needs of both automotive and multimedia applications, namely very high strength along with moderately high conductivity, in particular, the alloys of the preferred embodiments of the present invention are capable of being processed to strip products with combinations of yield strength / electrical conductivity of at least about 140 ksi (965 MPa) with a conductivity of at least about 30% IACS.

The alloys of the preferred embodiment of the present invention, have an improved combination of yield strength and electrical conductivity, good stress relaxation resistance, along with modest levels of bendability. Where an optimum level of yield strength and electrical conductivity is needed, e.g. a combination of 140 ksi (965 MPa) YS / 30% IACS, the composition is given in claim 1. Generally, excessive coarse second phases are present when alloying elements are substantially beyond the indicated upper limits.

The electrical conductivity and yield strength of the alloy are highest when the (Ni+Co)/(Si-Cr/5) ratio is controlled between about 3.5 and about 5. The ratio of Ni/Co is optimal for yield strength and conductivity when controlled between about 3 and about 5.

Magnesium generally increases stress relaxation resistance and softening resistance in the finished products; it also increases softening resistance during in-process aging annealing heat treatments. When present at low levels, Sn generally provides solid solution strengthening and also increases softening resistance during in-process aging annealing heat treatments, without excessively harming conductivity. Low levels of Mn generally improve bend formability, although with a loss of conductivity.

The preferred embodiment of the process of the present invention comprises melting and casting; hot rolling from 750° to 1050°C, optional milling to remove oxide, and an optional homogenization or intermediate bell anneal, cold rolling to a convenient gauge for solutionizing, solution annealing treatment at 800°- 1050°C for 10 seconds to one hour followed by a quench or rapid cool to ambient temperature to obtain an electrical conductivity of less than about 20% IACS (11.6 MS/m) and an equiaxed grain size of about 5-20 µm; a 0 to 75% cold rolling reduction in thickness; an age hardening anneal at 300 - 600°C from 10 minutes to 10 hours; and subsequently a further cold rolling 10 to 75% reduction in thickness to finish gauge; and second age hardening anneal at 250 to 500°C for 10 minutes to 10 hours. The resulting alloy can also be processed to finish gauge without using an in-process solutionizing heat treatment by using cycles of lower temperature bel! annealing treatments with intervening cold work. In addition, one or more optional recrystallization anneal(s) may be added to the process during the reduction from hot roiled gauge to the thickness appropriate for solutionizing.

The preferred scheme to result in alloy with a yield strength of at least about 140 ksi (965 MPa), and a conductivity of at least about 30% IACS conductivity involves solutionizing at about 900°t o 1000°C, cold rolling by about 25%, aging at about 450°- 500°C for 3 - 9 hours, c old rolling by about 20 - 25% to finish gauge, and aging 300°- 350°C for 3 -9 hours .

While this disclosure is particularly drawn to a process for the manufacture of copper alloy strip, the alloys of the invention and the processes of the invention are equally amenable to the manufacture of other copper alloy products, such as foil, wire, bar and tube. In addition, processes other than conventional casting, such as strip casting, powder metallurgy and spray casting are also within the scope of the invention.

The alloys and methods of the preferred embodiments will be better understood from the following illustrative examples:

### Example 1 - Increasing Alloy Levels Increases Strength; Cobalt Substitution Improves Both Strength and Conductivity

A series of ten pound (4.5 Kgs) laboratory ingots with the compositions listed in Table 2 were melted in a silica crucible and Durville cast into steel molds, which after gating were approximately 4" X 4" X 1.75" (0,1 m X 0,1 m X 0,044 m). Fig. 1 is a flow chart of the process of this Example 1. After soaking two hours at 900°C they were hot rolled in three passes to 1.1" (28 mm) (1.6" / 1.35" /1.1") (41 mm / 34 mm / 28 mm), reheated at 900°C for 10 minutes, and further hot rolled in three passes to 0.50" (13 mm) (0.9" / 0.7" / 0.5") (23 mm / 18 mm / 13 mm), followed by a water quench, followed by a homogenization or over-aging anneal at 590° for 6 hours. After trimming and milling to rem ove the surface oxide, the alloys were cold rolled to 0.012" (0,3 mm) and solution heat treated in a fluidized bed furnace for the time and temperature listed in Table 2. Time and temperature were selected to achieve approximately constant grain size. The alloys were then subjected to an aging anneal of 400° to 500°C for 3 hours, designed to increase strength and conductivity. The alloys were then cold rolled 25% to 0.009" (0,23 mm) and aged at 300° to 400°C for 4 hours. Properti es measured after the second age anneal are presented in Table 3. The data indicate that yield strength increases with increasing alloying levels in the ternary alloys J994 through J999, from 127 to 141 ksi (876 to 972 MPa) yield strength when Si levels range from 0.8 to 1.3%, respectively. Comparing J994, K001 and K002 to examine the effect of Co on alloys near 0.8% Si, the substitution of Co for Ni increases both yield strength and conductivity. Considering a Co substitution for Ni in alloys with ∼1.2%Si, K003 shows a decrease in yield strength and an increase in conductivity, while K004 shows an increase in yield strength and decrease in conductivity when compared to J998.

Having a Ni/Co ratio of about 3 (K002 and K004) leads to a higher strength than a Nt/Co ratio of 1 (K001 and K003), particularly at the higher Si level. Mn alloys K011 and K012 show evidence that Mn substitution for Ni improves the strength/bend properties, but at a significant loss of conductivity. Sn appears to provide solid solution strengthening, when comparing J994 to K036 and K037.

| **Table 2 - Alloys of Examples 1 and 2** | | | |
|---|---|---|---|
| Alloy | Analyzed composition, wt% | Solution Anneal conditions | Grain Size, µm |
| J994 | Cu - 3.33 Ni - 0.81 Si | 850°C - 1 minute | 11.2 |
| J995 | Cu - 3.78 Ni - 0.92 Si | 900°C -1 minute | 16.5 |
| J996 | Cu - 4.17 Ni - 1.03 Si | 900°C - 1 minute | 22.1 |
| J997 | Cu - 4.48 Ni - 1.12 Si | 900°C - 1 minute | 22.1 |
| J998 | Cu - 4.88 Ni - 1.24 Si | 900°C - 1 minute | 12.9 |
| J999 | Cu - 5.39 Ni -1.35 Si | 900°C - 2 minute | 14.1 |
| K001 | Cu - 1.65 Ni - 0.82 Si - 1.66 Co | 1000°C - 30 seconds | 12.9 |
| K002 | Cu - 2.56 Ni - 0.80 Si - 0.79 Co | 950°C - 1 minute | 17.7 |
| K003 | Cu - 2.45 Ni - 1.23 Si - 2.46 Co | 1000°C - 30 seconds | 6.7 |
| K004 | Cu - 3.70 Ni - 1.22 Si - 1.15 Co | 1000°C - 30 seconds | 12.9 |
| K009 | Cu - 1.74 Ni - 0.78 Si - 1.67 Mn | 850°C - 30 seconds | 28.2 |
| K010 | Cu - 2.65 Ni - 0.79 Si - 0.79 Mn | 850°C - 30 seconds | 22.1 |
| K011 | Cu - 2.51 Ni - 1.19 Si - 2.56 Mn | 850°C - 1 minute | 9.1 |
| K012 | Cu - 3.70 Ni -1.21 Si - 1.19 Mn | 850°C -1 minute | 9.8 |
| K013 | Cu - 3.22 Ni - 0.81 Si - 0.10 Cr | 850°C - 1 minute | 12.6 |
| K014 | Cu - 3.31 Ni - 0.82 Si - 0.18 Cr | 850°C - 1 minute | 10.7 |
| K015 | Cu - 4.82 Ni - 1.21 Si - 0.09 Cr | 900°C - 1 minute | 15.5 |
| K016 | Cu - 4.89 Ni - 1.26 Si - 0.18 Cr | 900°C - 1 minute | 12.9 |
| K036 | Cu - 3.69 Ni - 0.73 Si - 0.52 Sn | 850°C - 2 minute | 10.3 |
| K037 | Cu - 3.66 Ni - 0.77 Si - 0.93 Sn | 850°C - 2 minute | 16.2 |
| K040 | Cu - 3.74 Ni - 0.72 Si - 0.08 Mg | 850°C - 2 minute | 17.7 |
| K041 | Cu - 3.78 Ni - 0.76 Si - 0.205 Mg | 850°C - 2 minute | 18.8 |

| **Table 3 Properties of the Alloys from Examples 1 from SA-age-CR-age process** | | | | |
|---|---|---|---|---|
| Alloy | Ages | %IACS | YS/TS/EI ksi/ksi/% | 90° MBR/t |
| J994 | 450/300 | 36.8 | 126.7/130.8/2 | 2.9/3.4 |
| J995 | 450/300 | 35.5 | 130.8/134.7/1 | 3216.7 |
| J996 | 450/300 | 34.5 | 132.7/138.5/2 | 3.1/6.9 |
| J997 | 450/300 | 33.7 | 135.3/139.3/2 | 3.7/6.7 |
| J998 | 450/300 | 34.3 | 137.9/144.2/2 | 3.3/8.6 |
| J999 | 450/300 | 34.2 | 140.9/147.1/2 | 3.4/6.7 |
| K001 | 500/300 | 40.3 | 129.2/134.4/2 | -- |
| K002 | 500/350 | 40.5 | 130.3/135.8/2 | 3.8/5.2 |
| K003 | 450/300 | 37.8 | 129.7/134.3/2 | 3.5/3.7 |
| K004 | 450/300 | 28.4 | 145.3/150.8/2 | 5.1/6.8 |
| K009 | 450/350 | 16.5 | 108.1/113.3/4 | -- |
| K010 | 450/300 | 22.9 | 127.1/131.3/2 | -- |
| K011 | 400/300 | 11.9 | 137.6/141.0/2 | 2.4/3.2 |
| K012 | 400/300 | 17.0 | 135.41140,412 | 2.4/3.7 |
| K013 | 450/300 | 36.7 | 125.41129-6/2 | -- |
| K014 | 450/300 | 36.2 | 128.0/131.9/2 | -- |
| K015 | 450/300 | 33.8 | 135.6/139.8/2 | 3.5/5.2 |
| K016 | 450/300 | 32.4 | 136.0/140.4/2 | 3.3/5.2 |
| K036 | 450/300 | 34.3 | 131.5/143.1/1 | 3.9/6.9 |
| K037 | 450/300 | 30.8 | 135.2/147.1/2 | 3.5/6.8 |
| K040 | 450/350 | 38.4 | 125.4/136.5/2 | -- |
| K041 | 450/350 | 37.7 | 123.7/135.5/1 | -- |

### Example 2 - Cobalt Improves Strength

Selected alloys of Example 1 were solution heat treated in a fluidized bed furnace for the time and temperature listed in Table 2. Fig. 2 is a flow chart of the process of this Example 2. Subsequently the alloys were cold rolled 25 % to 0.009" (0,23 mm) then subjected to an aging anneal of 400° to 500°C for 3 hours. After an additional cold reduction of 22% to 0.007" (0,18 mm), samples were aged annealed at temperatures of 300° to 400°C for 3 hours. Properties from representative conditions are listed in Table 4. Bend properties in many cases are somewhat better at similar strengths than the process in Example 1. Co (K003 and K004) and Sn (K037) additions provide the highest strength increase of the alloys in this example.

| **Table 4 Properties of the Alloys from Examples 2 from SA-CR-age-CR-age process** | | | | |
|---|---|---|---|---|
| Alloy | Ages | %IACS | YS/TS/EI ksi/ksi/% | 90° MBR/t |
| J994 | 450/300 | 38.3 | 130.0/134.3/2 | 2.3/3.7 |
| J997 | 450/300 | 37.7 | 125.2/132.7/2 | 2.9/8.9 |
| J998 | 400/300 | 28.8 | 128.4/134.0/2 | 3.1/4.0 |
| J999 | 400/300 | 29.5 | 131.9/135.4/2 | 3.1/5.1 |
| K002 | 450/300 | 35.1 | 125.0/129.2/1 | 2.4/4.9 |
| K003 | 450/300 | 33.7 | 135.2/140.3/2 | 3.1/4.0 |
| K004 | 450/300 | 31.9 | 134.4/139.7/2 | 3.7/6.7 |
| K014 | 450/300 | 38.1 | 127.9/132.3/2 | 2.3/4.0 |
| K036 | 450/300 | 36.0 | 129.2/131.8/1 | 3.1/3.9 |
| K037 | 450/300 | 32.0 | 135.2/139.8/2 | 3.3/4.7 |
| K040 | 450/300 | 38.7 | 127.1/129.3/1 | -- |
| K041 | 450/300 | 38.4 | 132.4/136.4/1 | 3.6/4.7 |

### Example 3 - Cobalt and Chromium Levels and (Ni+Co)/(Si-Cr/5) Ratio

A series of ten (4.5 Kgs) laboratory ingots with the compositions listed in Table 5 were melted in a silica crucible and Durville cast into steel molds, which after gating were approximately 4" X 4"X 1.75" (0,1 m X 0,1 m X 0,044 m). Figure 3 is a flow chart of the process of this Example 3. After soaking two hours at 900°C they were hot roiled in three passes to 1.1" (28 mm) (1.6" / 1.35" / 1.1") (41 mm / 34 mm / 28 mm), reheated at 900°C for 10 minutes, and further hot rolled in three passes to 0.50" (13 mm) (0.9" / 0.7" / 0.5") (23 mm / 18 mm / 13 mm), followed by a water quench. The quenched plates were then soaked at 590°C for 6 hours, trimmed and then milled to remove surface oxides developed during hot rolling. The alloys were then cold rolled to 0.012" (0,3 mm) and solution heat treated in a fluidized bed furnace for 60 seconds at the temperatures listed in Table 5. The temperature was selected to maintain a fairly constant grain size. Alloys were then subjected to an aging anneal of 400° to 500°C for 3 hours, designed to increase strength and conductivity. The alloys were then cold rolled 25% to 0.009" (0,23 mm) and aged at 300° to 400°C for 4 hours. Properties measured after the second age anneal are presented in Table 6. From this data set, it can be observed that additions to a base Alloy of Cu-Ni-Si of Co (K068), Cr (K072), or both Co and Cr (K070) achieve the best combinations of strength, conductivity and bend formability. It is also noted that relatively high Si levels of 1.2% and above were present in the samples with the highest strength. While there was some evidence of strengthening from Sn, this was accompanied by poor bend formability. in Table 5, it can be seen that the ratio (Ni+Co)/(Si-Cr/5) is very close to 4 for most of the alloys, particularly K068, K070 and K072. Also, the Ni/Co ratio was close to 3 for K068 and K070. Yield strength is plotted against conductivity in Figure 4, and against bend formability in Figure 5. The values for K068, K070 and K072 are identified to show their unusually good combination of properties.

| **Table 5 Alloys of Examples 3 and 4** | | | | | |
|---|---|---|---|---|---|
| Alloy | Analyzed composition, wt% | <Ni+Co)/(Si-Cr/5)Ratio | Ni/Co | Solution Anneal Temperature | Grain Size, µm |
| K056 | Cu - 4.94 Ni - 0.97 Si - 0.86 Sn | 5.09 | | 900°C | 15 |
| K057 | Cu - 2.63 Ni - 0.73 Co - 0.80 Si - 0.88 Sn | 4.20 | 3.60 | 925°C | 16 |
| K058 | Cu - 3.80 Ni - 0.97 Co - 1.24 Si - 0.83 Sn | 3.85 | 3.92 | 950°C | 14 |
| K059 | Cu - 3.27 Ni - 0.82 Si - 0.22 Mn | 3.99 | | 850°C | 20 |
| K061 | Cu - 3.83 Ni - 128 Co - 1.27 Si - 0.31 Mn | 4.02 | 2.99 | 950°C | 8 |
| K065 | Cu - 4.96 Ni - 125 Si - 0.085 Mg | 3.97 | | 900°C | 17 |
| K066 | Cu - 3.29 Ni - 0.84 Si - 0.33 Mn - 0.092 Mg | 3.92 | | 850°C | 10 |
| K087 | Cu - 2.57 Ni - 0.83 Co - 0.83 Si - 0.082 Mg | 4.10 | 3.10 | 950°C | 21 |
| K068 | Cu - 3.80 Ni - 1.21 Co - 1.27 Si - 0.048 Mg | 3.94 | 3.14 | 975°C | 12 |
| K069 | Cu - 3.42 Ni - 0.84 Si 0.89 Sn - 0.062 Mg | 4.07 | | 875°C | 28 |
| K070 | Cu - 3.83 Ni - 1.29 Co - 1.39 Si - 0.56 Cr | 4.01 | 2.97 | 975°C | 8 |
| K071 | Cu - 3.36 Ni - 0.95 Si - 0.54 Cr - 0.035 Mg | 3.99 | | 950°C | 19 |
| K072 | Cu - 4.64 - Ni - 1.28 Si - 0.54 Cr - 0.078 Mg | 3.96 | | 950°C | 17 |
| K073 | Cu - 3.52 Ni - 1.07 Si - 1.06 Cr - 0.047 Mg | 4.10 | | 950°C | 14 |
| K074 | Cu - 4.11 Ni - 1.31 Si - 1.01 Cr - 0.058 Mg | 3.71 | | 975°C | 18 |
| K075 | Cu - 4.71 Ni - 1.29 Si - 0.50 Cr - 0.85 Sn | 3.96 | | 950°C | 19 |
| K076 | Cu - 3.54 Ni - 1.00 Si - 0.49 Cr - 0.89 Sn | 3.92 | | 925°C | 17 |

| **Table 6 Properties from SA-age-CR-age process of Example 3** | | | | |
|---|---|---|---|---|
| Alloy | Ages | %IACS | YS/TS/EI ksi/ksi/% | 90° MBR/t |
| K056 | 450/300 | 25.7 | 142.7/148.4/2 | 8.7/8.7 |
| K057 | 450/350 | 29.0 | 131.3/137.6/3 | 3.3/6.9 |
| K058 | 450/300 | 24.5 | 142.8/149.0/2 | 5.2/6.9 |
| K059 | 450/350 | 32.2 | 132.3/137.5/3 | 2.9/2.9 |
| K061 | 450/350 | 27.2 | 142.0/146.5/2 | 3.6/5.2 |
| K065 | 450/300 | 32.4 | 137.8/143.1/1 | 6.9/6.9 |
| K066 | 450/350 | 29.1 | 134.5/139.8/2 | 3.1/3.1 |
| K087 | 500/300 | 38.6 | 132.4/137.0/2 | 3.8/5.2 |
| K068 | 450/300 | 28.6 | 143.2/149.3/2 | 4.0/6.9 |
| K069 | 450/350 | 30.3 | 134.1/139.4/3 | 4.0/6.9 |
| K070 | 450/350 | 31.0 | 147.1/151.9/2 | 4.0/4.0 |
| K071 | 450/350 | 33.5 | 134.9/140.0/3 | 3.1/3.3 |
| K072 | 450/350 | 30.6 | 145.7/151.1/2 | 4.0/6.9 |
| K073 | 450/350 | 33.8 | 141.6/146.6/2 | 3.8/4.0 |
| K074 | 450/350 | 29.4 | 146.9/153.1/2 | 3.8/6.9 |
| K075 | 450/350 | 26.2 | 145.4/152.9/3 | 5.2/8.7 |
| K076 | 450/350 | 27.7 | 137.7/144.8/3 | 3.1/6.9 |

### Example 4 - Cobalt and Chromium for Strength and Formability

The alloys of Example 3 were solution heat treated in a fluidized bed furnace for 60 seconds at the temperature listed in Table 5. Figure 6 is a flow chart of the process of this Example 4. Subsequently the alloys were cold rolled 25 % to 0.009" (0,23 mm) then subjected to an aging anneal of 400° to 500°C for 3 hours. After an additional cold reducti on of 22% to 0.007" (0,18 mm), samples were aged annealed at temperatures of 300° to 400°C for 3 hours. Properties from representative conditions are listed in Table 7. Similar to Example 3, of particular note are alloys K068, K070 and K072, which show that alloys containing Co, Cr or a combination of both achieve the highest strength levels. The bend formability data indicates that K068 and K070 which both contain Co have the best formability at higher strength. Yield strength is plotted against conductivity in Figure 7, and against bend formability in Figure 8. The values for alloys K068, K070 and K072 are noted.

| **Table 7 Properties from SA-CR-age-CR-age process of the Alloys of Exhibit 4** | | | | |
|---|---|---|---|---|
| Alloy | Ages | %IACS | YS/TS/EI ksi/ksi/% | 90° MBR/t |
| K056 | 450/300 | 29.1 | 147.4/152.4/2 | 5.7/8.6 |
| K057 | 450/300 | 29.7 | 136.1/141.9/2 | 2.0/5.7 |
| K058 | 450/300 | 25.6 | 146.7/153.3/1 | 2.0/8.6 |
| K065 | 450/300 | 34.7 | 142.9/145.4/2 | 3.6/4.9 |
| K087 | 500/300 | 38.4 | 137.4/141.7/3 | 2.9/5.7 |
| K068 | 450/300 | 30.3 | 151.6/155.3/1 | 3.6/4.9 |
| K069 | 450/300 | 29.7 | 139.4/145.7/1 | 2.9/8.6 |
| K070 | 450/300 | 31.1 | 152.3/157.9/2 | 2.9/3.9 |
| K071 | 450/300 | 34.8 | 143.8/147.6/2 | 2.9/3.9 |
| K072 | 450/300 | 31.4 | 155.4/161.3/1 | 2.7/8.6 |
| K073 | 450/300 | 34.7 | 147.2/150.9/2 | 2.7/3.9 |
| K074 | 450/300 | 29.8 | 153.9/160.0/1 | 2.1/3.9 |
| K075 | 450/300 | 26.5 | 151.4/158.2/2 | 2.0/11.0 |
| K076 | 450/300 | 28.1 | 142.8/149.0/1 | 2.1/8.6 |

### Example 5 - Nickel : Cobalt Ratio

A series of ten pound (4.5 Kgs) laboratory ingots with the compositions listed in Table 8 were melted in a silica crucible and Durville cast into steel molds, which after gating were approximately 4" X 4" X 1.75" (0,1 m X 0,1 m X 0,044 m). Figure 9 is a flow chart of the process of this Example 5. This group of alloys was based on K068, K070 and K072 from Table 5, wherein overall alloying level and Ni/Co ratio were varied while keeping the stoichiometric ratio ((Ni+Co)/(Si-Cr/5)) close to 4.2. After soaking two hours at 900°C they were hot roiled in three passes to 1.1" (28 mm) (1.6" / 1.35" / 1.1") (41 mm / 34 mm / 28 mm), reheated at 900°C for 10 minutes, and further hot rolled in three passes to 0.50" (13 mm) (0.9" / 0.7" / 0.5") (23 mm / 18 mm / 13 mm), followed by a water quench. The quenched plates were then soaked at 590°C for 6 hours, trimmed and then milled to remove surface oxides developed during hot rolling. The alloys were then cold rolled to 0.012" (0,3 mm) and solution heat treated in a fluidized bed furnace for 60 seconds at the temperature listed in Table 8. The temperature was selected to maintain a fairly constant grain size. Alloys were then subjected to an aging anneal of 450° to 500°C for 3 hours, designed to increase strength and conductivity. The alloys were then cold rolled 25% to 0.009" (0,23 mm) and aged at 300 to 400°C for 4 hours. Properties measured after the second age anneal for the process with a 475°C first age and 300°C second age are presented in Table 9. For the Co-only set of compositions (K077 to K085), yield strength values tend to increase with higher alloying content. For example, K078, with a Ni+Co+Cr+Si value of 6.24, had a yield strength of 155 ksi (1069 MPa) while K084 with a Ni+Co+Cr+Si value of 5.22 had a 139 ksi (958 MPa) yield strength. A Ni/Co ratio of 3 to 4 provides better strength than a ratio of 5, when one compares K077 (Ni/Co ratio of 3.62) and K078 (Ni/Co ratio of 3.83) to K079 (Ni/Co ratio of 5.04), as well as comparing K080 (Ni/Co ratio of 3.32) and K081 (Ni/Co ratio of 3.93) to K082 (Ni/Co ratio of 4.89). The plots of yield strength vs Ni/Co ratio in Figure 10 illustrate this, with the exception of K085, which has a higher Si level than K083 and K084. The Co-and-Cr-containing alloys, K086 to K094, were not as sensitive to overall alloying levels and Ni/Co ratio as the Co-only alloys. The Cr-only alloys (K095 to K097) also had comparable properties to the other alloy types.

| **Table 8 Alloys of Example 5** | | | | | | |
|---|---|---|---|---|---|---|
| Alloy | Analyzed composition, wt% | Ni/Co | Nl+Co+Cr+Si | (Ni+Co)/(Si-Cr/5) Ratio | Solution Anneal Temperalure, °C | Grain Size, µm |
| K077 | Cu - 3.84 Ni - 1.06 Co - 1.31 Si | 3,62 | 6.21 | 3.740 | 975 | 10.0 |
| K078 | Cu - 3.98 Ni - 1.04 Co - 1.22 Si | 3.83 | 6.24 | 4.115 | 975 | 10.3 |
| K079 | Cu - 4.28 Ni - 0.85 Co - 1.32 Si | 5.04 | 6.45 | 3.886 | 975 | 14.8 |
| K080 | Cu - 3.49 Ni - 1.05 Co - 1.10 Si | 3.32 | 5.64 | 4.127 | 975 | 15.5 |
| K081 | Cu - 3.77 Ni - 0.96 Co - 1.17 Si | 3.93 | 5.90 | 4.043 | 975 | 16.9 |
| K082 | Cu - 3.86 Ni - 0.79 Co - 1.12 Si | 4.89 | 5.77 | 4.152 | 975 | 20.4 |
| K083 | Cu - 3.22 Ni - 1.05 Co - 1.06 Si | 3.07 | 5.33 | 4.028 | 975 | 15.5 |
| K084 | Cu - 3.33 Ni - 0.89 Co - 1.00 Si | 3.74 | 5.22 | 4.220 | 950 | 15.3 |
| K085 | Cu - 3.59 Ni - 0.75 Co - 1.16 Si | 4.79 | 5.50 | 3.741 | 950 | 18.7 |
| K086 | Cu - 3.80 Ni - 1.20 Co - 1.46 Si - 0.51 Cr | 3.17 | 7.03 | 3.715 | 975 | 10.9 |
| K087 | Cu - 4.03 Ni - 1.01 Co -1.37 Si - 0.60 Cr | 3.99 | 7.01 | 4.032 | 975 | 15.9 |
| K088 | Cu - 4.26 Ni - 0.82 Co - 1.51 Si - 0.57 Cr | 5.20 | 7.16 | 3.639 | 975 | 16.4 |
| K089 | Cu - 3.50 Ni - 1.110 Co - 1.33 Si - 0.58 Cr | 3.15 | 6.52 | 3.797 | 975 | 10.5 |
| K090 | Cu - 3.75 Ni - 0.92 Co - 1.25 Si - 0.55 Cr | 4.08 | 6.47 | 4.096 | 975 | 16.3 |
| K091 | Cu - 3.97 Ni - 0.79 Co - 1.42 Si - 0.56 Cr | 5.03 | 6.74 | 3.639 | 975 | 16.7 |
| K092 | Cu - 3.25 Ni - 1.01 Co - 1.22 Si - 0.58 Cr | 3.22 | 6.06 | 3.859 | 975 | 15.2 |
| K093 | Cu - 3.43 Ni - 0.86 Co - 1.90 Si - 0.51 Cr | 3.99 | 6.10 | 3.581 | 975 | 16.0 |
| K094 | Cu - 3.50 Ni - 0.73 Co - 1.22 Si - 0.59 Cr | 4.79 | 6.04 | 3.838 | 975 | 17.5 |
| K095 | Cu - 4.97 Ni - 1.36 Si - 0.60 Cr | | 6.93 | 4.008 | 950 | 18.4 |
| K096 | Cu - 4.63 Ni - 1.35 Si - 0.61 Cr | | 6.59 | 3.770 | 925 | 12.0 |
| K097 | Cu - 4.20 Ni - 1.18 Si - 0.59 Cr | | 5.97 | 3.955 | 925 | 18.9 |

| **Table 9 Properties from SA-age-CR-age process of Example 5** | | | | |
|---|---|---|---|---|
| Alloy | Ages | %IACS | YS/TS/EI ksi/ksi/% | 90° MBR/t |
| K077 | 475/300 | 29.1 | 152.1/159.3/4 | 5.2/5.2 |
| K078 | 475/300 | 29.7 | 155.5/162.3/4 | 5.2/5.2 |
| K079 | 475/300 | 30.7 | 143.7/150.1/4 | |
| K080 | 475/300 | 31.2 | 142.4/147.9/3 | 5.2/3.6 |
| K081 | 475/300 | 30.7 | 144.2/148.3/3 | 4.0/6.1 |
| K082 | 475/300 | 32.2 | 137.7/142.7/2 | |
| K083 | 475/300 | 31.1 | 140.0/145.8/3 | 5.2/5.2 |
| K084 | 475/300 | 32.1 | 138.9/145.6/3 | |
| K085 | 475/300 | 31.8 | 140.4/146.3/2 | |
| K086 | 475/300 | 30.1 | 151.6/157.9/4 | 5.2/6.1 |
| K087 | 475/300 | 30.5 | 149.4/153.6/3 | 5.2/3.6 |
| K088 | 475/300 | 30.4 | 152.2/159.3/4 | 5.2/5.2 |
| K089 | 475/300 | 30.3 | 149.0/155.6/3 | 4.0/5.2 |
| K090 | 475/300 | 31.3 | 161.9/157.4/3 | 5.2/3.8 |
| K091 | 475/300 | 30.7 | 149.5/154.5/3 | 5.2/6.1 |
| K092 | 475/300 | 30.8 | 146.5/152.1/3 | 4.0/5.2 |
| K093 | 475/300 | 30.3 | 147.2/153.4/4 | 5.2/5.2 |
| K094 | 475/300 | 31.2 | 148.1/154.4/2 | 4.0/3.8 |
| K095 | 475/300 | 30.7 | 150.2/159.1/3 | 3.8/6.1 |
| K096 | 475/300 | 32.1 | 153.3/160.6/4 | 4.0/6.1 |
| K097 | 475/300 | 31.9 | 148.7/155.5/3 | 3.8/5.2 |

The alloys of Table 8 were solution heat treated in a fluidized bed furnace 60 seconds at the temperature listed in Table 8. Subsequently the alloys were cold rolled 25 % to 0.009" (0,23 mm) then subjected to an aging anneal of 450 to 500°C for 3 hours. After an additional cold reduction of 22% to 0.007" (0,18 mm), samples were aged annealed at temperatures of 300 to 400°C for 3 hours. Properties from samples given first and second ages at 450°C and 300°C, respectively, are listed in Table 10. The Co -only alloys displayed a sensitivity to overall alloying levels with this scheme which was not found in alloys containing Cr. The only Co-only alloys at 150 ksi (1034 MPa) yield strength and above were K077 and K078, while all Cr-containing alloys reached or came close to that strength level. Strength-bend properties for this process are fairly similar to those in Table 9.

| **Table 10 Properties from SA-CR-age-CR-age process of Example 5** | | | | |
|---|---|---|---|---|
| Alloy | Ages | %IACS | YS/TS/EI ksi/ksi/% | 90° MBR/I |
| K077 | 450/300 | 29.1 | 152.8/160.2/2 | 3.7/4.3 |
| K078 | 450/300 | 30.1 | 149.7/157.7/4 | 4.0/4.9 |
| K079 | 450/300 | 35.2 | 133.4/140.3/2 | |
| K080 | 450/300 | 32.2 | 133.1/139.6/2 | |
| K081 | 450/300 | 32.2 | 133.0/138.8/2 | |
| K082 | 450/300 | 44.9 | 100.7/112.9/3 | |
| K083 | 450/300 | 30.2 | 140.7/145.8/3 | |
| K084 | 450/300 | 31.8 | 141.7/146.7/3 | 4.0/5.1 |
| K085 | 450/300 | 31.2 | 141.4/146.7/2 | |
| K086 | 450/300 | 30.3 | 150.8/156.6/2 | 4.9/6.7 |
| K087 | 450/300 | 302 | 153.4/158.7/2 | 4.6/4.9 |
| K088 | 450/300 | 28.6 | 153.7/159.4/2 | 3.7/6.7 |
| K089 | 450/300 | 29.8 | 148.9/155.4/1 | 4.6/6.7 |
| K090 | 450/300 | 29.9 | 151.3/155.9/3 | 4.6/4.3 |
| K091 | 450/300 | 30.0 | 152.4/159.5/1 | 4.0/6.7 |
| K092 | 450/300 | 32.5 | 149.6/156.4/3 | 4.3/6.7 |
| K093 | 450/300 | 30.3 | 147.1/152.7/2 | 4.6/6.7 |
| K094 | 450/300 | 29.9 | 160.4/156.9/2 | 4.3/4.9 |
| K095 | 450/300 | 30.0 | 155.9/165.3/2 | 4.0/6.7 |
| K096 | 450/300 | 31.8 | 157.5/165.4/3 | 4.0/6.7 |
| K097 | 450/300 | 32.0 | 155.1/161.6/3 | 4.3/4.9 |

### Example 6 - Nickel: Cobalt Ratio

Laboratory ingots with the compositions listed in Table 11 were melted in a graphite crucible and Tamman cast into steel molds, which after gating were 4.33" X 2.17"X1.02" (110 mm X 55 mm X 26 mm). Figure 11 is a flow chart of the process of this Example 6. For a target Si-content of 1% and Cr-content of 0.5% one alloy is Co-containing and the other is Co-free, the Ni-content is adjusted in order to keep a stoichiometric ratio ((Ni+Co)/(Si-Cr/5)) of close to 4.2. After soaking two hours at 900°C they were hot rolled to 0.472" (12 mm), thereby reheated after each pass at 900°C for 10 mi nutes. After the last pass the bar was water quenched. After trimming and milling to 0.394" (10 mm) in order to remove the surface oxide, the alloys were cold rolled to 0.0106" (0,27 mm) and solution heat treated in a fluidized bed furnace for the time and temperature listed in Table 11. Time and temperature were selected to achieve grain sizes below 20µm. The alloys were then subjected to an aging anneal of 450 to 500°C for 3 hours, designed to increase strength and conductivity. The alloys were then cold rolled 25 % to 0.0079" (0,2 mm) and aged at 300 or 400°C for 3 hours. Properties measured after the second age anneal are presented in Table 12. The formability was measured via V-block. The data indicates that both alloys are capable of achieving a yield strength of 135 ksi (931 MPa), yet the Co-containing variant BS shows a better softening resistance that can be seen with increasing the age annealing temperature. The slightly better bad way bendability of variant BS is presumably due to the slightly lower grain size after solution annealing.

| **Table 11 Alloys of Example 6, wt.%** | | | | | | | | | |
|---|---|---|---|---|---|---|---|---|---|
| alloy | Ni | Co | Cr | Si | Mg | (Ni+Co)/(Si-Cr/5) Ratio* | Ni/Co | SA conditions | Grain size, *µ*m |
| BR | 3.59 | | 0.48 | 1.00 | | 3.97 | ∞ | 915°C - 1 minute | 10-15 |
| BS | 3.18 | 0.47 | 0.49 | 0.97 | | 4.19 | 6.77 | 950°C - 1 minute | 5-10 |

| **TABLE 12 Properties from SA-age-CR-age Process of Example 6** | | | | | | | | | | | |
|---|---|---|---|---|---|---|---|---|---|---|---|
| Alloy | 1.AA | 2.AA 300°C/3h | | | | | 2AA 400°C/3h | | | | |
| | Temp °C | YS ksi | TS ksi | A10% | %IACS | 90° MINBR/ | YS ksi | TS ksi | A10% | %IACS | 90° MINBR/ |
| BR | 450 | 135.8 | 144.2 | 3.7 | 32.5 | 4.0/5.0 | 118.2 | 129.5 | 6.5 | 37.1 | -/- |
| | 475 | 133.9 | 141.8 | 3.7 | 35.1 | 4.0/6.0 | 124.0 | 132.9 | 7.9 | 38.5 | -/- |
| | 500 | 117.3 | 123.6 | 5 | 37.1 | 4.0/4.0 | 100.1 | 108.8 | 11 | 41.6 | -/- |
| BS | 450 | 135.8 | 142.6 | 1.8 | 31.7 | 4.0/4.0 | 128.2 | 137.2 | 3.7 | 33.5 | 3.5/4.0 |
| | 475 | 132.7 | 138.4 | 1.7 | 34.6 | 5.0/5.5 | 126.5 | 136.2 | 2.3 | 38.3 | 4.0/4.5 |
| | 500 | 127.3 | 134.7 | 4.8 | 37.4 | 4.0/5.0 | 119.4 | 127.8 | 6 | 41.2 | -/- |

### Example 7 - (Ni+Co)/(Si-Cr/5) Ratio

A group of alloys was cast and processed using once more the basic compositions of K068 (Co only), K070 (Co and Cr) and K072 (Cr only) from Table 5 as a base, but in this case with a gradual drop in Si levels, thus increasing the (Ni+Co)/(Si-Cr/5) stoichiometric ratio above the 3.6 to 4.2 range of previous alloys. Ni and Co levels were designed to be constant for each of the three alloy types. A series of ten pound laboratory ingots with the compositions listed in Table 11 were melted in a silica crucible and Durville cast into steel molds, which after gating were approximately 4" X 4" X 1.75" (0,1 m X 0,1 m X 0,044 m). K143 to K146 are variants of K072, K160 to K163 variants of K070, and K164 to K167 are variants of K068. Figure 12 is a flow chart of the process of this Example 7. After soaking two hours at 900°C they were hot rolled in three passes to 1.1" (28 mm) (1.6" / 1.35" / 1.1") (41 mm / 34 mm / 28 mm), reheated at 900°C for 10 minutes, and further hot roiled in three passes to 0.50" (13 mm) (0.9" / 0.7" / 0.5") (23 mm / 18 mm / 13 mm), followed by a water quench. The quenched plates were then soaked at 590° C for 6 hours, trimmed and then milled to remove surface oxides developed during hot rolling. The alloys were then cold rolled to 0.012" (0,3 mm) and solution heat treated in a fluidized bed furnace for 60 seconds at the temperatures listed in Table 13. The temperature was selected to maintain a fairly constant grain size. The alloys were then cold rolled 25% to 0.009" (0,23 mm) and aged 450, 475 and 500°C for 3 hours. Properties aft er each aging temperature for alloys of the current example, as well as K068, K070, K072, K078, K087 and K089 are listed in Table 14. For each alloy type, yield strength decreases as the stoichiometric ratio increases above about 4.5, and falls below 120 ksi (827 MPa) at a ratio of around 5.5. This is shown in Figures 13 to 15 for the Cr alloys (plus K072 data), the Co-alloys (plus K068 and K078 data), and the Co-Cr alloys (plus K070, K087 and K089 data), respectively. In the Co and Cr alloys, conductivity decreases as the stoichiometric ratio increases above about 4.5, while for the alloys with both Co and Cr there is not a clear relationship between stoichiometry and conductivity. This is shown graphically in Figures 16 through 18. Based on this data it is evident that the best yield strength-conductivity properties are produced when the stoichiometric ratio is kept between 3.5 and 5.0.

| **Table 13 Alloys of Example 7** | | | | | | | | |
|---|---|---|---|---|---|---|---|---|
| alloy | Ni | Co | Cr | Si | Mg | (Ni+Co)/(Si-Cr/5) Ratio | Ni/Co | SA Temperature |
| K143 | 4.61 | | 0.519 | 1.11 | 0.099 | 4.582 | | 950 |
| K144 | 4.63 | | 0.503 | 0.828 | 0.074 | 6.365 | | 950 |
| K145 | 4.59 | | 0.607 | 0.91 | 0.085 | 5.820 | | 950 |
| K146 | 4.55 | | 0.576 | 0.803 | 0.093 | 6.615 | | 950 |
| K160 | 3.84 | 1.2 | 0.52 | 1.19 | | 4.641 | 3.20 | 975 |
| K161 | 3.8 | 1.18 | 0.515 | 1.1 | | 4.995 | 3.22 | 975 |
| K162 | 3.83 | 1.2 | 0.513 | 1.03 | | 5.424 | 3.19 | 975 |
| K163 | 3.84 | 1.21 | 0.556 | 0.938 | | 6.108 | 3.17 | 975 |
| K164 | 3.74 | 1.17 | | 1.05 | 0.104 | 4.676 | 3.20 | 975 |
| K165 | 3.9 | 1.23 | | 1.01 | 0.116 | 5.079 | 3.17 | 975 |
| K166 | 3.87 | 1.23 | | 0.918 | 0.12 | 5.556 | 3.15 | 975 |
| K167 | 3.9 | 1.24 | | 0.83 | 0.085 | 6.193 | 3.15 | 975 |

| **Table 14 Properties after solution annexing, cold rolling 25% and aging of Example 7** | | | | | | | | | |
|---|---|---|---|---|---|---|---|---|---|
| alloy | 450°C age | | | 475°C age | | | 500°C age | | |
| | YS, ksi | %IACS | 90° bends | YS, ksi | %IACS | 90° bends | YS, ksi | %IACS | 90° bends |
| K143 | 138.9 | 31.2 | 2.9/2.0 | 135.8 | 33.7 | 2.0/2.7 | 126.3 | 35.8 | 2.0/2.2 |
| K144 | 118.1 | 27.5 | 1.8/2.2 | 125.6 | 30.8 | 1.3/1.1 | 121.3 | 33.1 | 22/1.3 |
| K145 | 120.8 | 27.3 | 2.0/1.3 | 127.5 | 30,3 | 2.2/1.3 | 123.5 | 32.6 | 2.2/1.8 |
| K146 | 113.4 | 26.8 | 1.8/1.1 | 121.7 | 30.4 | 2.2/2.0 | 116.8 | 32.2 | 1.3/1.6 |
| K160 | 127.4 | 29.5 | 2.0/3.1 | 133.8 | 34.0 | 2.4/1.6 | 122.6 | 39.3 | 1.8/1.8 |
| K161 | 127.4 | 29.4 | 2.4/1.1 | 131.3 | 33.0 | 2.2/1.6 | 123.5 | 35.7 | 1.8/0.7 |
| K162 | 122.4 | 33.4 | 1.3/1.3 | 120.7 | 34.4 | 2.4/1.3 | 116.5 | 35.9 | 1.6/1.3 |
| K163 | 120.7 | 29.8 | 1.3/1.1 | 119.4 | 32.0 | 1.6/1.1 | 111.1 | 34.2 | 1.6/1.1 |
| K164 | 126.6 | 29.9 | 2.4/1.6 | 132.6 | 33.7 | 2.4/2.0 | 125.8 | 36.7 | 2.0/2.9 |
| K165 | 118.9 | 29.6 | 2.2/1.6 | 124.0 | 32.9 | 2.2/2.4 | 119.5 | 35.4 | 1.6/1.8 |
| K166 | 116.6 | 27.9 | 2.0/1.3 | 120.4 | 30.4 | 2.9/1.1 | 117.7 | 32.5 | 2.0/1.8 |
| K167 | 111.6 | 25.7 | 2.0/1.6 | 114.5 | 27.4 | 1.6/1.3 | 113.4 | 29.3 | 1.3/0.2 |
| K068 | 131.9 | 29.3 | 2.2/2.8 | | | | 131.7 | 33.5 | 2.2/2.2 |
| K070 | 134.7 | 29.7 | 2.2/1.6 | | | | 129.7 | 33.6 | 1.7/1.6 |
| K072 | 133.3 | 29.9 | 1.7/1.7 | | | | 130.0 | 33.2 | 1.6/2.2 |
| K078 | 125.3 | 30.8 | -- | 133.3 | 31.9 | 2.2/1.6 | 125.7 | 36.3 | -- |
| K087 | 133.4 | 29.0 | -- | 136.9 | 30.7 | 2.2/1.6 | 124.1 | 37.7 | -- |
| K089 | 136.2 | 29.9 | -- | 135.0 | 30.6 | -- | 131.5 | 34.4 | -- |

### Example 8 - (Ni+Co)/(Si-Cr/5) Ratio

A series of ten pound (4.5 Kgs) laboratory ingots with the compositions listed in Table 15 were melted in a silica crucible and Durville cast into steel molds, which after gating were approximately 4" X 4" X 1.75" (0,1 m X 0,1 m X 0,044 m). Figure 19 is a flow chart of the process of this Example 8. After soaking two hours at 900°C they were hot rolled in three passes to 1.1" (28 mm) (1.6" / 1.35" / 1.1") (41 mm / 34 mm / 28 mm), reheated at 900°C for 10 minutes, and further hot rolled in three passes to 0.50" (13 mm) (0.9" / 0.7" / 0.5") (23 mm / 18 mm / 13 mm), followed by a water quench. The quenched plates were then soaked at 590°C for 6 hours, trimmed and then milled to remove surface oxides developed during hot rolling. The alloys were then cold rolled to 0.012" (0,3 mm) and solution heat treated in a fluidized bed furnace for 60 seconds at 950°C. Grain size ranged from 6 to 12 µm. Alloys were then subjected to an aging anneal of 450 or 475°C for 3 hours, designed to increase strength and conductivity. The alloys were then cold rolled 25 % to 0.009" (0,18 mm) and aged at 300°C f or 4 hours. Properties measured after the second age anneal are presented in Table 16.

Table 17 has properties measured after samples were solution heat treated in a fluidized bed furnace for 60 seconds at 950°C, cold rolled 25% to 0.009" (0,23 mm), given an aging anneal at 475°C fo r 3 hours, cold rolled 22% to 0.007" (0,18 mm), and given a final anneal of 300°C for 3 hours. The results show the viability of a range of compositions with Si from 1.0 to 1.2%, with a Ni/Co ratio of 4, and a stoichiometric ratio (((Ni+Co)/(Si-Cr/5))) of 3.5 to 5.0. This is shown graphically in Figures 20 and 21, which plot conductivity and yield strength data from Table 17 versus the stoichiometric ratio. These plots show yield strengths of 140 ksi (965 MPa) or higher combined with conductivities of 25 %IACS or higher are obtained for this process when the ratio is between 3.0 and 5.0. Cr was not found to influence properties significantly in the alloys of this example.

Stress relaxation tests were run on samples of K188 and K205 which were cold rolled to 0.012" (0,3 mm) from milled hot rolled plate, solution annealed at 950°C for 60 seconds, cold rolled 25% to 0.009" (0,23 mm), and age annealed at 475°C for 3 hours. The stress relaxation tests were run at 150°C for 3000 hours on samples of longitudinal and transverse orientation. Results in Table 18 show that both alloys had excellent stress relaxation resistance, over 85% stress remaining after 1000 hours at 150°C, regardl ess of Cr content or sample orientation.

| **Table 15 Alloys of Example 8** | | | | |
|---|---|---|---|---|
| Alloy | Analyzed composition, wt% | Ni/Co | Stoichiometric ratio | Grain Size, µm |
| K188 | Cu - 3.40 Ni - 0.81 Co - 1.16 Si - 0.42 Cr - 0.019 Mg | 4.20 | 3.91 | 7.3 |
| K189 | Cu - 3.20 Ni - 0.72 Co - 1.05 Si - 0.38 Cr - 0.033 Mg | 4.46 | 4.02 | 10.1 |
| K190 | Cu - 3.22 Ni - 0.70 Co - 1.28 Si - 0.31 Cr - 0.036 Mg | 4.59 | 3.22 | 8.5 |
| K191 | Cu - 3.22 Ni - 0.70 Co - 1.05 Si - 0.53 Cr - 0.064 Mg | 4.58 | 4.16 | 9.5 |
| K192 | Cu - 2.94 Ni - 0.69 Co - 1.29 Si - 0.55 Cr - 0.062 Mg | 4.24 | 3.08 | 10.9 |
| K193 | Cu - 3.21 Ni - 0.90 Co - 1.05 Si - 0.34 Cr - 0.117 Mg | 3.56 | 4.18 | 8.6 |
| K194 | Cu - 3.20 Ni - 0.84 Co - 1.30 Si - 0.22 Cr - 0.035 Mg | 3.80 | 3.22 | 7.8 |
| K195 | Cu - 3.18 Ni - 0.86 Co - 0.81 Si - 0.52 Cr - 0.070 Mg | 3.71 | 5.72 | 7.1 |
| K196 | Cu - 3.19 Ni - 0.89 Co - 1.28 Si - 0.57 Cr - 0.111 Mg | 3.60 | 3.49 | 7.7 |
| K197 | Cu - 3.61 Ni - 0.70 Co - 1.06 Si - 0.36 Cr - 0.067 Mg | 5.14 | 4.36 | 10.7 |
| K198 | Cu - 3.60 Ni - 0.70 Co - 1.28 Si - 0.39 Cr - 0.077 Mg | 5.13 | 3.58 | 8.7 |
| K199 | Cu - 3.60 Ni - 0.70 Co - 1.06 Si - 0.60 Cr - 0.076 Mg | 5.13 | 4.58 | 9.3 |
| K200 | Cu - 3.60 Ni - 0.70 Co - 1.28 Si - 0.60 Cr - 0.092 Mg | 5.14 | 3.70 | 9.3 |
| K201 | Cu - 3.63 Ni - 0.88 Co - 1.04 Si - 0.29 Cr - 0.065 Mg | 4.12 | 4.59 | 6.0 |
| K202 | Cu - 3.62 Ni - 0.90 Co - 1.27 Si - 0.36 Cr - 0.101 Mg | 4.04 | 3.77 | 7.4 |
| K203 | Cu - 3.59 Ni - 0.89 Co - 1.05 Si - 0.56 Cr - 0.076 Mg | 4.04 | 4.77 | 6.1 |
| K204 | Cu - 3.58 Ni - 0.88 Co - 1.27 Si - 0.56 Cr - 0.075 Mg | 4.09 | 3.85 | 5.9 |
| K205 | Cu - 3.73 Ni - 0.91 Co - 1.13 Si - 0.082 Mg | 4.09 | 4.11 | 12.1 |
| K206 | Cu - 3.53 Ni - 0.81 Co - 1.02 Si - 0.080 Mg | 4.36 | 4.25 | 12.2 |
| K207 | Cu - 3.53 Ni - 0.78 Co -1.25 Si - 0.055 Mg | 4.55 | 3.44 | 9.9 |
| K208 | Cu - 3.57 Ni - 1.00 Co - 1.02 Si - 0.070 Mg | 3.57 | 4.48 | 7.6 |
| K209 | Cu - 3.54 N - 1.02 Co - 1.25 Si - 0.085 Mg | 3.47 | 3.65 | 7.4 |
| K210 | Cu - 3.94 N - 0.82 Co - 1.06 Si - 0.149 Mg | 4.78 | 4.49 | 9.5 |
| K211 | Cu - 3.97 Ni - 0.80 Co - 1.24 Si - 0.085 Mg | 4.97 | 3.85 | 11.5 |
| K212 | Cu - 3.95 Ni - 0.99 Co - 1.04 Si - 0.100 Mg | 4.01 | 4.75 | 10.2 |
| K213 | Cu - 3.97 Ni - 0.99 Co - 1.22 Si - 0.079 Mg | 4.01 | 4.07 | 10.2 |

| **Table 16 SA-age-CR-age process properties of Example 8** | | | | |
|---|---|---|---|---|
| Alloy | Ages | %IACS | YS/TS/EI ksi/ksi/% | 90° MBR/t |
| K188 | 450/300 | 29.3 | 149.5/156.1/2 | 3.3/5.2 |
| K189 | 475/300 | 33.6 | 147.3/153.8/2 | 4.0/4.0 |
| K204 | 450/300 | 29.7 | 149.6/155.1/2 | 4.0/5.2 |
| K205 | 475/300 | 34.2 | 149.8/155.7/2 | 4.0/5.2 |
| K206 | 475/300 | 35.0 | 147.9/153.9/2 | 4.0/5.3 |
| K213 | 475/300 | 34.2 | 150.8/157.4/2 | 5.2/5.2 |

| **Table 17 SA-CR-age-CR-age process properties of Example 8** | | | | |
|---|---|---|---|---|
| Alloy | Ages | %IACS | YS/TS/EI ksi/ksi/% | 90° MBR/t |
| K188 | 475/300 | 35.1 | 145.7/152.4/3 | 2.0/4.9 |
| K189 | 475/300 | 34.7 | 146.1/152.6/2 | 2.6/5.7 |
| K190 | 475/300 | 28.0 | 139.2/148.5/4 | 2.9/5.1 |
| K191 | 475/300 | 37.2 | 143.7/149.9/3 | 3.4/6.7 |
| K192 | 475/300 | 28.1 | 139.7/146.4/2 | 2.6/6.7 |
| K193 | 475/300 | 36.2 | 143.6/149.3/3 | 2.9/5.1 |
| K194 | 475/300 | 29.1 | 138.7/146.1/3 | 2.6/6.7 |
| K195 | 475/300 | 35.5 | 130.7/134.7/4 | 2.0/3.4 |
| K196 | 475/300 | 30.2 | 143.4/149.5/2 | 2.6/9.0 |
| K197 | 475/300 | 35.4 | 145.3/152.0/2 | 3.1/6.7 |
| K198 | 475/300 | 31.7 | 148.2/155.7/3 | 2.9/6.7 |
| K199 | 475/300 | 35.5 | 147.8/154.4/3 | 2.9/9.0 |
| K200 | 475/300 | 33.7 | 146.3/152.9/3 | 3.4/6.7 |
| K201 | 475/300 | 36.8 | 145.2/150.0/2 | 2.9/6.7 |
| K202 | 475/300 | 33.5 | 146.1/152.8/3 | 2.6/5.1 |
| K203 | 475/300 | 34.4 | 147.4/153.6/2 | 3.6/5.7 |
| K204 | 475/300 | 33.9 | 150.3/156.8/3 | 2.9/6.7 |
| K205 | 475/300 | 35.3 | 147.0/152.8/2 | 2.9/5.7 |
| K206 | 475/300 | 35.8 | 146.9/153.7/3 | 2.4/6.7 |
| K207 | 475/300 | 29.7 | 143.3/150.3/2 | 2.6/6.7 |
| K208 | 475/300 | 36.2 | 142.5/148.1/3 | 2.9/6.7 |
| K209 | 475/300 | 32.2 | 145.5/152.1/3 | 2.6/6.7 |
| K210 | 475/300 | 34.1 | 148.6/154.1/5 | 2.9/6.7 |
| K211 | 475/300 | 33.8 | 144.7/152.1/2 | 3.1/5.1 |
| K212 | 475/300 | 34.5 | 140.6/145.4/3 | 2.9/5.7 |
| K213 | 475/300 | 35.0 | 148.4/154.4/2 | 3.6/6.7 |

| **Table 18 150°C Stress Relaxation Data for samples cold rolled 25% and aged at 475°C for 3 hours of Example 8** | | | | | |
|---|---|---|---|---|---|
| Alloy | Yield Strength, ksi | Longitudinal | | Transverse | |
| | | (in percent stress remaining) | | (in percent stress remaining) | |
| | | 1000 hr 3000hr | | 1000 hr | 3000 hr |
| K188 (Cr) | 136.4 | 89.9 | 87.9 | 88.2 | 85.2 |
| | | | | | |
| K205 (no Cr) | 132.2 | 92.0 | 90.4 | 91.6 | 89.6 |

### Example 9 - Effect of Cr

A series of ten pound laboratory ingots with the compositions listed in Table 19 were melted in a silica crucible and Durville cast into steel molds, which after gating were approximately 4" X 4" X 1.75" (0,1 m X 0,1 m X 0,044 m). Figure 22 is a flow chart of the process of this Example 9. The ingots were then machined to have tapered edges, as illustrated schematically in Figure 23, to create a higher state of tensile stress at the edges. This condition is more prone to edge cracking than the standard flat edges, and thus more sensitive to alloying additions, in this case Cr. The alloys were soaked for two hours at 900°C, and rolled in two passes to 1.12" (28,4 mm) (1.4" / 1.12") (35,6 mm / 28,4 mm) then water quenched. After examination for cracks, the bars were reheated at 900°C for two hours, and rolled in three passes to 0.50" (13 mm) (0.9" / 0.7" / 0.5") (23 mm / 18 mm / 13 mm), followed by a water quench. It was found that without Cr, K224 developed large cracks during the first few passes of hot rolling, which enlarged during the remaining passes. None of the Cr-containing alloys developed large cracks during hot roiling. A few of the alloys showed small cracks after initial passes believed to be due to casting defects, but these did not enlarge during subsequent passes. The Cr effect was the same independent of Cr level, from 0.11% to 0.55%. Examples of edge conditions of K224 and K225 after hot rolling are shown in Figures 24 and 25. The addition of even a small amount of Cr would reduce cracking in plant production, thus improving yield after hot rolling and coil milling. Data from plant-cast bars (i.e., bars cast as pilot product dc castings), whose compositions are listed in Table 20, show the beneficial effect of Cr on preventing hot rolling cracks and therefore improving yield. Table 21 lists the normalized casting plant yield (CPY) of six Cr-containing and four non-Cr bars, where the normalized CPY is obtained as follows: First the individualized CPY is calculated as the ratio of coil milled weight to cast bar weight. Second the bar with the highest CPY, in this case RN 033410, is assigned a normalized CPY of 100%. Third the normalized CPY of all other bars is calculated by dividing the CPY of each bar by the CPY of RN033410. The normalized CPY of bars without Cr is 48-82% compares to 82-100% for the Cr-containing bars.

Limiting the Cr level would be desirable due to the abrasiveness of Cr-silicides, which is demonstrated in Figure 26. Figure 26A shows wear on a tool steel ball which was slid for 3000 linear inches (76 m) (1500 inches (38 m) on each side of the strip) under a 100 gm load over the strip surface with lard oil as a lubricant of a non-Cr sample (RN033407) that was plant solution annealed at 975°C, cold rolled 25% then aged a 450° C and sulfuric acid cleaned, while Figure 26B has a similar condition using a sample of a Cr-containing alloy (RN834062). The polished appearance of the ball shown in Fig. 26 shows that the Cr-containing alloy caused much more wear, leading to a significantly larger volume of material being removed from the ball. This is seen in Fig. 26 as a much larger wear scar for the Cr-containing alloy. The larger wear scar suggests that during stamping of a sheet of the alloy into parts, a high amount of tool wear would occur.

| **Table 19 Alloys used in Example 9** | | | | | |
|---|---|---|---|---|---|
| Alloy | Ni | Co | Cr | Si | Mg |
| K224 | 3.71 | 0.91 | 0 | 1.14 | -- |
| K225 | 3.71 | 0.93 | 0.11 | 1.19 | 0.030 |
| K226 | 3.61 | 0.82 | 0.23 | 1.20 | 0.035 |
| K227 | 3.50 | 0.95 | 0.34 | 1.20 | 0.035 |
| K228 | 3.51 | 0.85 | 0.46 | 1.21 | 0.040 |
| K229 | 3.39 | 0.85 | 0.55 | 1.20 | 0.043 |

| **Table 20 Compositions of plant-cast bars of Example 9** | | | | | |
|---|---|---|---|---|---|
| Bar | Ni | Co | Cr | Si | Mg |
| RN032037 | 3.71 | 0.75 | -- | 1.09 | 0.12 |
| RN032038 | | | | | |
| RN033407 | 3.66 | 0.88 | -- | 1.07 | 0.106 |
| RN033408 | | | | | |
| RN033409 | 3.83 | 0.89 | 0.45 | 1.22 | 0.138 |
| RN033410 | | | | | |
| RN834059 | 3.24 | 0.758 | 0.425 | 1.02 | 0.094 |
| RN834060 | | | | | |
| RN834061 | 3.45 | 0.74 | 0.44 | 1.14 | 0.076 |
| RN834062 | | | | | |

| **Table 21 Milling data for plant-cast bars of Example 9** | | |
|---|---|---|
| Bar | Type | CPY% (NORMALIZED) |
| RN032037 | Non Cr | 75.2% |
| RN032038 | Non Cr | 48.1% |
| RN033407 | Non Cr | 76.0% |
| RN033408 | Non Cr | 82.3% |
| RN033409 | Cr | 95.6% |
| RN033410 | Cr | 100% |
| RNB34059 | Cr | 92.1% |
| RNB34060 | Cr | 90.1% |
| RN834061 | Cr | 87.7% |
| RN834062 | Cr | 82.0% |
| | | |

A Single casting run produced three bars with the composition shown in Table 21a. Casting plant yield of the bars, which was normalized similarly to the data of Table 21 where RN033410 is considered 100%, is given in Table 21b. The CPY of the low-Cr bars compares favorably with the Cr-containing bars of Table 21. This is believed to be due to Cr reducing cracking during hot rolling even at these low levels. RN037969 has a normalized CPY% above 100 due to the fact that the yield of this bar was higher than RN033410 in the earlier example.

| **Table 21a Analyzed compositions of low-Cr bars cast and processed in the plant** | | | | | |
|---|---|---|---|---|---|
| Bar | Ni | Co | Cr | Si | Mg |
| 037969 | 3.70 | 0.98 | 0.059 | 1.07 | 0.093 |
| 037970 | | | | | |
| 037971 | | | | | |

| **Table 21b** | | |
|---|---|---|
| Bar | Type | CPY% (normalized) |
| RN037969 | Low-Cr | 102.1% |
| RN037970 | Low-Cr | 89.8% |
| RN037971 | Low-Cr | 68.4% |

### Example 10 - Effect of Cr, Mn

A series of ten pound (4.5 Kgs) laboratory ingots with the compositions listed in Table 22 were melted in a silica crucible and Durville cast into steel molds, which after gating were approximately 4" X 4" X 1.75" (0,1 m X 0,1 m X 0,044 m). Figure 27 is a flow chart of the process of this Example 10. Alloy K259 contains a smaller level of Cr than those alloys in Example 9, to investigate the lower limits of the beneficial effect of Cr on hot rolling. Alloys K251, K254 and K260 contain low levels of Mn, to determine if Mn affects hot rollability in the alloy of this invention. The ingots were then machined to have tapered edges, as illustrated schematically in Fig. 23, to create a higher state of tensile stress at the edges. The alloys were soaked for two hours at 900°C, and roll ed in two passes to 1.12" (28,4 mm) (1.4" / 1.12") (35,6 mm / 28,4 mm) then water quenched. After examination for cracks, the bars were reheated at 900°C for two hours, and rolled in three passes to 0.50" (13 mm) (0.9" / 0.7" / 0.5") (23 mm / 18 mm / 13 mm), followed by a water quench. K259, with 0.058% Cr, hot rolled without edge crack formation. The Mn-containing alloys, along with K261 (with neither Cr nor Mn) developed large edge cracks. Thus a Cr addition near 0.05%, with a preferred range of 0.025 to 0.1% Cr, appears to be appropriate to balance hot reliability and formation of abrasive particles that would lead to tool wear.

The quenched bars were then soaked at 590s C for 6 hours, trimmed and then milled to remove surface oxides developed during hot rolling. The alloys were then cold rolled to 0.012" (0,3 mm) and solution heat treated in a fluidized bed furnace for 60 seconds at 950°C. Alloys were then subjected to an aging anneal of 475°C for 3 hours, designed to increase strength and conductivity. The alloys were then cold rolled 25 % to 0,009" (0,23 mm) and aged at 300°C for 3 hours. Alternatively, after solution heat treatment the alloys were cold rolled 25% to 0.009" (0,23 mm), given an aging anneal at 475°C for 3 hours, cold roiled 22% to 0.007" (0,18 mm), and given a final anneal of 300°C for 3 hours. Properties after the final age for both process paths are listed in Table 23. For both processes, the exceptionally good property combination of 150 ksi (1034 MPa) yield strength and at least 31 % IACS are achieved, with low levels of Cr, Mn or neither. Conductivity and yield strength are plotted in Figures 28 and 29 against the stoichiometric ratio ((Ni+Co)/(Si-Cr/5)) along with data from example 8 to demonstrate the unusually good properties reached when the ratio is kept between 3.0 and 5.0.

| **Table 22 Low Cr and Mn alloys of Example 10** | | | | | | | |
|---|---|---|---|---|---|---|---|
| Alloy | Ni | Co | Si | Mg | Cr | Mn | Ratio* |
| K251 | 3.64 | 0.84 | 1.16 | 0.058 | -- | 0.026 | 3.862 |
| K254 | 3.73 | 0.90 | 1.16 | 0.044 | -- | 0.061 | 3.991 |
| K259 | 3.78 | 0.56 | 1.14 | 0.073 | 0.058 | 0.004 | 3.846 |
| K260 | 3.75 | 0.94 | 1.15 | 0.065 | <.001 | 0.048 | 4.078 |
| K261 | 3.79 | 0.95 | 1.16 | 0.054 | <.001 | 0.004 | 4.086 |

| | | | | | | | |
|---|---|---|---|---|---|---|---|
| * Ratio = (Ni+Co)/(Si-Cr/5) | | | | | | | |

| **Table 23 Properties for Example 10** | | | | | | |
|---|---|---|---|---|---|---|
| Alloy | SA-age-CR-age process | | | SA-C R-age-CR-age process | | |
| | %IACS | YS/TS/EI | 90° MRB/t | %IACS | YS/TS/EI | 90° MBR/t |
| K251 | 31.0 | 149.9/156.5/1 | 4.0/52 | 32.0 | 151.9/158.6/3 | 2.6/2.9 |
| K254 | 33.7 | 141.2/144.7/2 | 3.3/3.3 | 33.0 | 151.7/158,1/1 | 2.3/3.7 |
| K259 | 31.8 | 151.0/157.3/2 | 4.0/5.2 | 33.3 | 150.8/156.9/2 | 2.3/2.9 |
| K260 | 32.4 | 149.9/156.3/3 | 3.8/3.8 | 35.3 | 148.6/154.7/3 | 2.9/4.3 |
| K261 | 31.9 | 150.9/157.1/2 | 3.8/5.2 | 34.4 | 151.0/157.6/2 | 2.6/4.3 |

### Example 11 - Effect of Processing

Sections of plant cast bar RN032037, whose composition is in Table 20, were processed from plant hot rolled and coil milled plate 0.600" (15,24 mm) thick. Samples were further processed by a variety of processing paths shown in Fig. 30. Process A involved cold rolling to 0.012" (0,3 mm) and solution heat treating in a fluidized bed furnace for 60 seconds at 950°C, age annealing at 500°C for 3 hours, cold roiling 25% to 0.009" (0,23 mm), and giving a second anneal at 350°C for 4 hours. In process BF the metal was rolled to 0.050" (1,3 mm) and given an intermediate bell anneal ("IMBA") of 575°C for 8 hours. Then the samples were subject to cold rolling to 0.012" (0,3 mm) and solution heat treating in a fluidized bed furnace for 60 seconds at 950°C, age annealing at 500°C for 3 hours, cold rolling 25% to 0.009" (0,23 mm), and giving a second anneal at 350°C for 4 hours. In process C, the allo y was rolled to 0.024" (0,61 mm) and solution heat treated in a fluidized bed furnace for 60 seconds at 950°C, followed by cold rolling to 0.012" (0,3 mm) and a second solution heat treatment in a fluidized bed furnace for 60 seconds at 950°C. Su bsequently, the process involved age annealing at 500°C for 3 hours, cold rolling 25% to 0.009" (0,23 mm), and giving a second anneal at 350°C for 4 hours. In process D, cold rolling to 0.012" (0,3 mm) was followed by solution heat treatment in a fluidized bed furnace for 60 seconds at 950°C the alloy was cold rolled 2 5% to 0.009" (0,23 mm), given an aging anneal at 475°C for 3 hours, cold rolled 22% to 0.007" (0,18 mm), and given a final anneal of 300°C for 3 hours. In proce ss E, the metal was rolled to 0.050" (1,27 mm) and given an intermediate bell anneal of 575°C for 8 hours. Then the samples were rolled to 0.024" (0,61 mm) and solution heat treated in a fluidized bed furnace for 60 seconds at 950°C, foil owed by cold rolling to 0.012" (0,3 mm) and a second solution heat treatment in a fluidized bed furnace for 60 seconds at 950°C. Subsequently, the process involved age annealing at 500°C for 3 hours, cold rolling 25% to 0.009" (0,23 mm), and giving a second anneal at 350°C for 4 hours.

| **Table 24 Properties resulting from the processes of Example 11** | | | | |
|---|---|---|---|---|
| Process | Description | YS/TS/EI | %IACS | 90° MBR/t |
| A | "Standard" process | 145.1/152.7/3 | 36.2 | 4.0/7.0 |
| B | IMBA process | 144.4/150.4/3 | 37.4 | 3.8/4.0 |
| C | Double solution anneal process | 147.2/152.7/3 | 37.1 | 3.6/6.9 |
| D | SA-CR-age-CR-age process | 146.5/154.4/2 | 34.2 | 4.2/8.7 |
| E | IMBA-double SA process | 143.6/150.1/3 | 36.7 | 3.3/7.0 |

### Example 12 Effect of Processing

Sections of plant cast bar RN032037, whose composition is in Table 20, were processed from plant hot rolled and coil milled plate 0.600" (15,24 mm) thick. Process variables were systematically varied to explore a matrix containing ranges of processing conditions. Figure 31 is a flow chart of the process of this Example 12. After cold rolling to 0.012" (0,3 mm), samples were solution annealed in a fluidized bed furnace at temperatures of 925, 950, 975 and 1000°C for 60 seconds. Coupons were then given age anneals at temperatures of 450, 475, 500 and 525°C for three hours. Samples we re then cold rolled to final thickness at varying reductions of 15, 25 and 35%. Finally, samples were given a second age anneal for four hours at 300, 325, 350 and 375°C. Table 25 contains properties of samples with different solution anneal temperatures while the rest of the process was held constant. As solution temperature is increased, yield strength increases, while conductivity decreases. Additionally, bend formability worsens at the higher solution annealing temperatures, due to the large grain size developed during the 975 and 1000°C anneals. Thus a solution annealed grain size below 20 µm is preferred.

When the temperature of the first age is varied while the other processing variables are held constant, it is found that the highest strength levels are due to the intermediate aging temperatures, as shown for the 475 and 500°C ages in Table 26. Also, the conductivity increased with increasing aging temperature. Thus the first age temperature can be manipulated to provide various desirable combinations of strength and conductivity.

When the roll reduction between the first and second ages was varied, yield strength was found to increase with increasing reduction, in this case up to 35%, while conductivity was unaffected. A larger increase in strength was found when going from 15 to 25% reduction than when going from 25 to 35%. Bend formability was found to worsen with higher reductions. The roll reduction can be manipulated to affect the strength-formability characteristics of the material produced. Use of roll reduction above 35% may be useful to produce peak strength, albeit with poorer formability.

Table 28 shows that the second age anneal temperature does not have a large effect on properties when the other processing variables are held constant. Conductivity was found to increase as the temperature of the second age increased, but to a small degree. Thus a wide operating range is acceptable for this step of the process.

| **Table 25 Effect of varying solution anneal temperatures, with 475°C first age, 25% roll reduction, 350°C second age of Example 12** | | | | |
|---|---|---|---|---|
| SA temperature, °C | SA grain size, µm | YS/TS/EI | %IACS | 90° Bends |
| 925 | 9.0 | 142.3/147.7/3 | 36.0 | 6.0/6.0 |
| 950 | 12.9 | 145.9/152.3/3 | 34.1 | 6.1/6.1 |
| 975 | 26.1 | 146.5/152.6/2 | 32.3 | 6.1/12.1 |
| 1000 | 28.8 | 147.5/152.1/3 | 32.7 | 8.7/12.1 |

| **Table 26 Effect of varying first age temperatures, with 950°C solution anneal, 25% roll reduction, 350° C second age of Example 12** | | | |
|---|---|---|---|
| 1^{st} Age Temp, °C | YS/TS/EI | %IACS | 90° Bends |
| 450 | 140.1/145.2/4 | 30.5 | 4.0/6.1 |
| 475 | 145.9/152.3/3 | 34.1 | 6.1/6.1 |
| 500 | 145.1/152.7/3 | 36.2 | 4.0/7.0 |
| 525 | 133.2/134.5/1 | 39.9 | n/m * |

| | | | |
|---|---|---|---|
| *not measured | | | |

| **Table 27 Effect of varying roll reductions, with 950°C solution anneal, 475°C first age, 350°C second age** | | | |
|---|---|---|---|
| Roll reduction | YS/TS/EI | %IACS | 90° Bends |
| 15% | 138.4/145.0/4 | 33.9 | 5.4/5.4 |
| 25% | 145.9/152.3/3 | 34.1 | 6.1/6.1 |
| 35% | 148.9/155.5/3 | 34.0 | 7.1/10.0 |

| **Table 28 Effect of varying second age temperatures, with 950°C solution anneal, 475°C first age, 25% roll reduction** | | | |
|---|---|---|---|
| 2^{nd} Age Temp, °C | YS/TS/EI | %IACS | 90° Bends |
| 300 | 146.4/152.0/2 | 33.2 | 6.1/6.1 |
| 325 | 146.5/152.3/3 | 33.6 | 6.1/8.7 |
| 350 | 145.9/152.3/3 | 34.1 | 6.1/6.1 |
| 375 | 146.2/152.7/3 | 34.8 | 6.0/8.6 |

Samples from the Cr-free plant-cast bar RN033407 (composition in Table 20) were rolled in the laboratory from the coil milled condition at 0.460" (11,7 mm) down to 0.012" (0,3 mm). Subsequently samples were solution heat treated in a fluidized bed furnace for 60 seconds at 900°C. Coupons were then rolled 25% to 0.009" (0,23 mm) and age annealed at 425, 450 and 475°C for times of 4 and 8 hours at each temperature. Subsequently samples were cold rolled 22% to 0.007" (0,18 mm) and given a final anneal of 300°C for three hours. The best combination of strength and conductivity resulted from the 450°C for 8 hour age, with the properties from that condition and others listed in Table 28a. Comparing the 450°C/8 hr data to the properties in Table 25, it is clear that further reducing the solution annealing temperature to 900°C lowers the yield strength and increases conductivity to produce the unique combination of 140 ksi (965 MPa) and 39 %IACS. In addition, the processing including a 900°C solution annealing temperature produced improved bend formability when compared to processing involving higher solution anneal temperatures.

| **Table 28A Properties after processing which includes a 900°C solution anneal.** | | | | |
|---|---|---|---|---|
| 1^{st} age condition | SA grain size, µm | YS/TS/EI | %IACS | 90° Bends |
| 450°C/4 hr | 5.5 | 138.5/143.0/2 | 36.1 | 2.6/4.0 |
| 450°C/8 hr | 5.5 | 140.3/144.7/2 | 39.0 | 2.0/4.3 |
| 475°C/4 hr | 5.5 | 126.9/131.7/3 | 40.7 | 2.3/4.0 |
| 475°C/8 hr | 5.5 | 131.0/135.0/3 | 41.2 | 1.7/2.3 |

### Example 13 - Effect of Si and Mg

Laboratory ingots with the compositions listed in Table 29 were melted in a graphite crucible and Tamman cast into steel molds, which after gating were 4.33" X 2.17" X 1.02" (110 mm X 55 mm X 26 mm). All alloys were targeted to have a Cr-content of 0.5%. The Si-content was varied between 1.0% and 1.5%. For the high-Si 1.5% variants the Ni/Co ratio was varied between 4.98 and 11.37 with a fixed stoichiometric ratio ((Ni+Co)/(Si-Cr/5)) around 4. The influence of Mg was tested by alloy BW with the same alloy composition as BV but with additionally 0.1% Mg.

Figure 32 is a flow chart of the process of this Example 13. After soaking two hours at 900°C they were hot roll ed to 0.472" (12 mm), thereby reheated after each pass at 900°C for 10 minutes. After the last pass the bar was water quenched. After trimming and milling to 0.394" (10 mm) in order to remove the surface oxide, the alloys were cold rolled to 0.012" (0,3 mm) and solution heat treated in a fluidized bed furnace for the time and temperature listed in Table 29. Time and temperature were selected to achieve grain sizes below 20 µm.

Subsequently the alloys were cold rolled 25 % to 0.009" (0,23 mm) then subjected to an aging anneal of 450 and 475°C for 3 hours. Properties of samples are listed in Table 30. The formability was measured via V-block. With increasing Si-content the yield strength is increasing from 121 ksi (834 MPa) for the 1.05% Si alloy to 135 ksi (931 MPa) for the 1.51% Si alloy. For the 1.16% Si variants Mg results in a benefit to yield strength of 5-7 ksi (34 - 48 MPa). Lowering the Ni/Co ratio from 11.37 to 4.98 enhances yield strength for the high Si (1.5%) alloys. Stress relaxation was tested by the ring method with a target initial stress of 0.8 times yield strength. Table 31 shows the stress relaxation data for variants BV, BW and BX. Comparing BV and BW, due to Mg addition the stress relaxation resistance increases from 66.3% to 86.6% for the 150°C/1000 h condition and from 48.5% to 72.3% for the 200°C/1000 h condition. The stress relaxation resistance of the higher Si-containing BX amounts to 82.3% for the 150°C/1000 h condition and 68.7% for the 200°C/1000 h condition.

**Table 29 Alloys of Examples 13 and 15, wt%**

| alloy | Ni | Co | Cr | Si | Mg | Ratio* | Ni/Co | SA conditions | Grain size, *µ*m |
|---|---|---|---|---|---|---|---|---|---|
| BU | 3,08 | 0,69 | 0,57 | 1,05 | | 4,03 | 4,46 | 950°C - 1 minute | 10-15 |
| BV | 3,51 | 0,75 | 0,49 | 1,16 | | 4,01 | 4,68 | 950°C - 1 minute | 10-15 |
| BW | 3,52 | 0,78 | 0,51 | 1,16 | 0,11 | 4,06 | 4,51 | 950°C - 1 minute | 15 |
| BT | 4,04 | 1,15 | 0,47 | 1,41 | | 3,94 | 3,51 | 975°C - 1 minute | 5 |
| BX | 4,89 | 0,43 | 0,50 | 1,48 | | 3,86 | 11,37 | 975°C - 1 minute | 15-20 |
| BY | 4,48 | 0,90 | 0,51 | 1,51 | | 3,82 | 4,98 | 975°C - 1 minute | 10 |

| | | | | | | | | | |
|---|---|---|---|---|---|---|---|---|---|
| *) Ratio = (Ni+Co)/(Si-Cr/5) | | | | | | | | | |

**Table 30 Properties from SA-Cr-AA Process of Example 13**

| Alloy | AA T, °C | YS, ksi | %IACS | 90° MINBR/t |
|---|---|---|---|---|
| BU | 450 | 121,0 | 27,6 | 2,2/1,3 |
| BV | 450 | 121,8 | 32,5 | 1,7/1,3 |
| | 475 | 120,5 | 34,8 | n.m. |
| BW | 450 | 126,9 | 31,8 | 2,2/2,6 |
| | 475 | 127,6 | 34,4 | n.m. |
| BT | 450 | 127,5 | 28,6 | n.m. |
| | 475 | 128,9 | 32,1 | n.m. |
| BX | 450 | 129,5 | 29,1 | 2,6/2,6 |
| | 475 | 125,9 | 31,1 | n.m. |
| BY | 450 | 135,2 | 30 | 2,2/2,2 |
| | 475 | 134,0 | 31,4 | 3,4/2,1 |

**Table 31 Stress Relaxation of Process SA - CR 25% - AA 450°C/3 h of Example 13**

| Alloy | YS, ksi | %IACS | remaining stress (%) | |
|---|---|---|---|---|
| | | | 150°C/1000h | 200°C/1000h |
| BV | 121.8 | 32.5 | 66.3 | 48.5 |
| BW | 126.9 | 31.8 | 86.6 | 72.3 |
| BX | 129.5 | 29.1 | 82.3 | 68.7 |

### Example 14 - Effect of Si and Mg

Figure 33 is a flow chart of the process of this Example 14. Specimens of Example 13 were subsequently cold rolled to 0.007" (0,18 mm) with a cold reduction of 22%. Thereafter the samples were aged annealed at temperatures of 300 °C to 400°C for 3 hours. Proper ties from samples given second ages at 300°C are listed in Table 32. The fo rmability was measured via V-block.

The highest yield strength was achieved with a first aging temperature of 450°C. With increasing Si-content th e yield strength is increasing from 131 ksi (903 MPa) for the Si 1.05% alloy to 147 ksi (1014 MPa) for the Si 1.51% alloy. For the Si 1.16% variants Mg results in a benefit to yield strength of 7-10 ksi (48 - 69 MPa). Lowering the Ni/Co ratio from 11.37 to 4.98 enhances yield strength for the high Si 1.5% alloys by 3 ksi (21 MPa). Stress relaxation was tested by the ring method with a target initial stress of 0.8 times yield strength. Table 33 shows the stress relaxation data for BV, BW and BX for the process SA - CR - 1 .AA 450°C - CR - 2.AA 300°C.

Comparing BV and BW, due to Mg addition the stress relaxation resistance increases from 72.6% to 85.6% for the 150°C/1000 h condition and from 55.8% to 69.3% for the 200°C/1000 h condition. The stress relaxation resistance of the higher Si-containing BX amounts to 81.1% for the 150°C/1000 h condition and 66.1% for the 200°C/1000 h condition.

**Table 32 Properties from SA-CR-1AA-CR-2AA Process of Example 14**

| Alloy | 1.AA T, °C | 2.AA 300°C/3h | | | | |
|---|---|---|---|---|---|---|
| | | YS, ksi | TS, ksi | A10, % | %IACS | 90° MINBR/t |
| BU | 450 | 130,7 | 138,1 | 2,6 | 33,6 | 5,5/5,5 |
| BV | 450 | 137,4 | 144,5 | 3,7 | 31,4 | 2,8/5,6 |
| | 475 | 130,8 | 137,8 | 4.8 | 34,8 | 2,8/5,0 |
| BW | 450 | 144,0 | 143,6 | 2,3 | 32,1 | 3,3/7,8 |
| | 475 | 141,3 | 147,1 | 3,8 | 34 | 2,8/6,7 |
| BT | 450 | 144,6 | 152,4 | 2,9 | 29,8 | 4,0/8,0 |
| | 475 | 137,8 | 146,2 | 4,2 | 34,1 | 4,0/7,0 |
| BX | 450 | 143,7 | 155,2 | 2,8 | 28,6 | 3,3/7,8 |
| | 475 | 134,4 | 148,2 | 2,8 | 31,2 | 2,8/6,7 |
| BY | 450 | 146,6 | 155,8 | 3 | 29,6 | 3,3/6,7 |
| | 475 | 137,8 | 150,0 | 4,3 | 32,2 | 3,3/6,7 |

**Table 33 Stress Relaxation Process SA-CR-1AA4500°C-C R-2AA300°C of Example 14**

| Alloy | YS, ksi | %IACS | remaining stress (%) | |
|---|---|---|---|---|
| | | | 150°C/1000h | 200°C/1000h |
| BV | 137.4 | 31.4 | 72.6 | 55.8 |
| BW | 144.0 | 32.1 | 85.6 | 69.3 |
| BX | 143.7 | 28.6 | 81.1 | 66.1 |

### Example 15: Effect of Si and Mg

Laboratory ingots with the compositions listed in Table 34 were melted in a graphite crucible and Tamman cast into steel molds, which after gating were 4.33" X 2.17" X 1.02" (110 mm X 55 mm X 26 mm). The alloys were Cr-free and with a stoichiometric ratio ((Ni+Co)/(Si-Cr/5)) around 4.2. The Ni/Co ratio was about 4.5. Two alloys have a targeted Si-content of 1.1%, but varying Mg-content and one alloy has an Si-content of 1.4% and additionally Mg. Figure 34 is a flow chart of the process of this Example 15. After soaking two hours at 900°C they were hot rolled to 0.472" (12 mm), there by reheated after each pass at 900°C for 10 minutes. After the last pass the bar w as water quenched. After trimming and milling to 0.394" (10 mm) in order to remove the surface oxide, the alloys were cold rolled to 0.012" (0,3 mm) and solution heat treated in a fluidized bed furnace for the time and temperature listed in Table 34. Time and temperature were selected to achieve grain sizes below 20 µm.

Subsequently the alloys were cold rolled 25 % to 0.009" (0,23 mm) then subjected to an aging anneal of 450 and 475°C for 3 hours. Properties of samples are listed in Table 35. The yield strength, formability measured with V-block and conductivity of the Cr-free FL and FM are similar to the Cr-containing BV and BW from Example 13, with comparable Si-content of 1.1%, Ni/Co ratio and stoichiometric ratio. As in Example 13, an addition of 0.1 %Mg results in a benefit to yield strength of 7-8 ksi (48 - 55 MPa).

With increasing Si-content from 1.17% to 1.39% the yield strength is increasing from 126.6 ksi (873 MPa) to 130.5 ksi (900 MPa) at the same solution annealing temperature. For variant FN, increasing the solution annealing temperature from 950°C to 1000°C results in an increase of yield strength of 10 ksi (69 MPa).

Stress relaxation was tested by the ring method with a target initial stress of 0.8 times yield strength. Table 36 shows the stress relaxation data for the processes with a solution annealing temperature of 950°C. Compared to the Cr-containing 1.16% Si samples of Example 13, BV and BW, the stress relaxation of FL and FM is slightly lower. Similar to Example 13, a Mg addition of 0.1% results in a stress relaxation increase from 64.6% to 82.7% for the 150°C/1000 h condition and from 44.3% to 69.2% for the 200°C/1000 h condition. The stress relaxation resistance of the Mg-containing, Si1.39% variant FN amounts to 84.1 % for the 150°C/1000 h condition an d 65.9% for the 200°C/1000 h condition.

| **Table 34 Alloys of Examples 15 and 16, wt.%** | | | | | | | | | |
|---|---|---|---|---|---|---|---|---|---|
| alloy | Ni | Co | Cr | Si | Mg | Ratio* | Ni/Co | SA conditions | Grain size, *µ*m |
| FL | 3.71 | 0.90 | | 1.09 | | 4.23 | 4.12 | 950°C - 1 minute | 10 |
| FM | 3.89 | 0.87 | | 1.17 | 0.10 | 4.05 | 4.47 | 950°C - 1 minute | 5-10 |
| FN | 5.19 | 0.99 | | 1.39 | 0.10 | 4.47 | 4.90 | 950°C - 1 minute | 10 |
| | | | | | | | | 1000°C - 1 minute | 15-20 |

| | | | | | | | | | |
|---|---|---|---|---|---|---|---|---|---|
| *) Ratio = (Ni+Co)/(Si-Cr/5) | | | | | | | | | |

**Table 35 Properties from SA-CR-AA Process of Example 15**

| Alloy | SA-conditions | AA T, °C | YS, ksi | %IACS | 90° MINBR/t GW/BW |
|---|---|---|---|---|---|
| FL | 950°C - 1 minute | 450 | 118.6 | 29.5 | 2.6/1.3 |
| | | 475 | 119.4 | 34.5 | 3.0/1.7 |
| FM | 950°C - 1 minute | 450 | 126.6 | 30.2 | 2.6/2.2 |
| | | 475 | 126 | 33.1 | 2.1/2.1 |
| FN | 950°C - 1 minute | 450 | 130.5 | 30.7 | 3.0/2.6 |
| | | 475 | 129.1 | 33.1 | 2.6/2.2 |
| | 1000°C - 1 minute | 450 | 141.7 | 27.1 | 3.5/3.9 |
| | | 475 | 139.2 | 29.6 | 3.5/4.8 |

**Table 36 Stress Relaxation of Process SA 950°C - CR 25% - AA 450°C/3 h of Example 15**

| Alloy | YS, ksi | %IACS | remaining stress (%) | |
|---|---|---|---|---|
| | | | 150°C/1000h | 200°C/1000h |
| FL | 118.6 | 29.5 | 64.6 | 44.3 |
| FM | 126.6 | 30.2 | 82.7 | 69.2 |
| FN | 130.5 | 30.7 | 84.1 | 65.9 |

### Example 16: Effect of Si and Mg

Figure 35 is a flow chart of the process of this Example 16. Specimens of Example 15 were subsequently cold roiled to 0.007" (0,18 mm) with a cold reduction of 22%. Thereafter the samples were aged annealed at temperatures of 300°C to 350°C for 3 hours. Properties from samples given second ages at 300°C are listed in Table 37. The fo rmability was measured via V-block. The highest yield strength was achieved with a first aging temperature of 450°C.

FM shows a higher yield strength of 11 ksi (76 MPa) in comparison to FL1 that is partly ascribed to the Mg-content and partly ascribed to the slightly higher Si-content. The yield strength, bendability and conductivity of the Cr-free FL and FM are similar to the Cr-containing BV and BW from example 15, with comparable Si-content, Ni/Co ratio and stoichiometric ratio.

Increasing Si-content from 1.17% to 1.39% leads to the same yield strength of about 144 ksi (993 MPa) for a solution annealing temperature of 950°C. For variant FN, increasing the solution anne aling temperature from 950°C to 1000°C results in an increase of yield strength from 143 ksi (986 MPa) to 158 ksi (1089 MPa).

Stress relaxation was tested by the ring method with a target initial stress of 0.8 times yield strength. Table 38 shows the stress relaxation data for FL and FM for the process SA 950°C - CR - 1 .AA 450°C -CR - 2.AA 300°C. Compared to the Cr-containing 1.16% Si samples of example 15, BV and BW, the stress relaxation of FL and FM is lower by 2-3%. Similar to example 15, a Mg addition of 0.1% results in a stress relaxation increase from 70.0% to 82.0% for the 150°C/1000 h condition and from 52.3% to 66.9% for the 200°C/1000 h condition. The stress relaxation resistance of the Mg-containing, Si 1.39% variant FN amounts to 85.0% for the 150°C/1000 h condition and 66.4% for the 200°C/1000 h condition.

**Table 37 Properties from SA-C R-1AA-C R-2 A A Process of Example 16**

| Alloy | SA-conditions | 1.AA T, °C | 2.AA 300°C/3h | | | | |
|---|---|---|---|---|---|---|---|
| | | | YS, ksi | TS, ksi | A10, % | %IACS | 90° MINBR/t GW/BW |
| FL | 950°C - 1 minute | 450 | 133.1 | 140 | 2.7 | 31.6 | 4.5/6.1 |
| | | 475 | 129.7 | 139.5 | 1.9 | 36.2 | 3.9/4.4 |
| FM | 950°C - 1 minute | 450 | 144 | 147.6 | 2 | 31 | 4.4/7.2 |
| | | 475 | 141.3 | 145 | 1.8 | 33.2 | 4.5/6.8 |
| FN | 950°C - 1 minute | 450 | 143.2 | 150.0 | 2 | 31.5 | 3.9/7.2 |
| | | 475 | 133.1 | 138.9 | 2.4 | 34.3 | 3.3/5.6 |
| | 1000°C - 1 minute | 450 | 158.1 | 165.1 | 1.4 | 27.6 | 6.0/9.4 |
| | | 475 | 157.5 | 164.6 | 1.9 | 30.9 | 4.418.3 |

**Table 38 Stress Relaxation of Process SA 950°C-CR-I AA 450°C-CR-2AA 300°C of Example 16**

| Alloy | YS, ksi | %IACS | remaining stress (%) | |
|---|---|---|---|---|
| | | | 150°C/1000h | 200°C/1000h |
| FL | 133.1 | 31.6 | 70.1 | 52.3 |
| FM | 144.0 | 31 | 82.0 | 66.9 |
| FN | 143.2 | 31.6 | 85.0 | 66.4 |

Figure 36 shows the relation between 90°-mi nBR/t BW and yield strength for the alloys and processes of Examples 13, 14, 15, and 16. Both processes SA-CR- AA and SA - CR - AA - CR - AA form two groups with a certain formability - yield strength relation. The solid lines are just a guide to the eye and mark increasing Min BR/t and increasing yield strength with higher Si-content and/or Mg-addition. There is almost no difference in yield strength and formability - yield strength relationship between the Cr-containing and Cr-free variants.

Figure 37 shows the relation between %IACS and yield strength for the alloys and processes of Examples 13, 14, 15, and 16. The Cr-free and the Cr-containing alloys show the same capability in achieving a conductivity of 30%iACS together with high yield strength. The SA - CR - AA - CR - AA process achieves higher yield strength than the SA-CR- AA process, but at the same conductivity.

## Claims

1. A copper base alloy having an improved combination of yield strength, electrical conductivity, stress relaxation resistance, consisting of:
between 3.5 and 3.9 weight percent Ni;
between 0.8 and 1.0 weight percent Co;
between 1.0 and 1.2 weight percent Si;
between 0.05 and 0.15 weight percent Mg;
up to 0.1 weight percent Cr;
up to 1.0 weight percent Sn, and up to 1.0 weight percent Mn,
the balance being copper and impurities, wherein the ration of Ni/Co is between 3 and 5, the alloy processed to have a yield strength of at least 140 ksi, and an electrical conductivity of at least 30% IACS.

2. The alloy according to claim 1 wherein the ratio of (Ni+Co)/(Si-Cr/5) is between 3.5 and 5.0.

3. A process for making a copper base alloy according to one of the preceding claims, comprising:
melting and casting the alloy;
hot rolling from 750° to 1050°C;
cold rolling to a convenient gauge for solutionizing;
solution annealing the alloy at between 800° and 1050°C for from 10 seconds to one hour; and
subsequently quenching or rapidly cooling the alloy to ambient temperature to obtain an electrical conductivity of less than 20% IACS (11.6 MS/m) and an equiaxed grain size of 5 - 20 µm;
cold rolling the alloy for a 0 to 75% reduction in thickness;
subjecting the alloy to an hardening anneal at 300° to 600°C for 10 minutes to 10 hours;
subsequently cold rolling the alloy for an 10 to 75% reduction in thickness to finish gauge;
subjecting the alloy to a second age hardening anneal at 250 to 500°C for 10 minutes to 10 hours.

4. The process according to claim 3 further comprising an intermediate recrystallization anneal after the hot rolling.

## Patentansprüche

1. Legierung auf Kupferbasis mit einer verbesserten Kombination aus Streckgrenze, elektrischer Leitfähigkeit und Spannungsrelaxationswiderstand, bestehend aus:
zwischen 3,5 und 3,9 Gewichtsprozent Ni;
zwischen 0,8 und 1,0 Gewichtsprozent Co;
zwischen 1,0 und 1,2 Gewichtsprozent Si;
zwischen 0,05 und 0,15 Gewichtsprozent Mg,
bis zu 0,1 Gewichtsprozent Cr;
bis zu 1,0 Gewichtsprozent Sn, und bis zu 1,0 Gewichtsprozent Mn,
wobei der Rest aus Kupfer und Verunreinigungen besteht und das Verhältnis von Ni / Co zwischen 3 und 5 liegt,
und wobei die Legierung derart bearbeitet wird, dass sie eine Streckgrenze von mindestens 140 ksi aufweist und die elektrische Leitfähigkeit mindestens 30% IACS beträgt.

2. Legierung nach Anspruch 1, **dadurch gekennzeichnet, dass** das Verhältnis von (Ni+Co)/(Si-Cr/5) zwischen 3,5 und 5,0 liegt.

3. Verfahren zur Herstellung einer Legierung auf Kupferbasis nach einem der vorhergehenden Ansprüche, umfassend folgende Schritte:
Schmelzen und Gießen der Legierung;
Warmwalzen von 750° auf 1050° C;
Kaltwalzen auf ein geeignetes Maß zum Lösungsglühen;
Lösungsglühen der Legierung zwischen 800° und 1050° C für 10 Sekunden bis zu einer Stunde; und
anschließendes Abschrecken oder schnelles Abkühlen der Legierung auf Umgebungstemperatur, um eine elektrische Leitfähigkeit von weniger als 20% IACS (11,6 MS/m) und einer gleichachsigen Korngröße von 5 - 20 Mikrometer zu erhalten;
Kaltwalzen der Legierung für eine Verringerung der Dicke um 0 bis 75%;
Unterziehen der Legierung einer Härtungsglühung bei 300 ° bis 600 ° für 10 Minuten bis 10 Stunden;
anschließendes Kaltwalzen der Legierung für eine Verringerung der Dicke um 10 bis 75% auf das Endmaß;
Unterziehen der Legierung einem zweiten Aushärtungsglühen bei 250 bis 500 ° C für 10 Minuten bis 10 Stunden.

4. Das Verfahren nach Anspruch 3, weiter umfassend ein Zwischenrekristallisationsglühen nach dem Warmwalzen.

## Revendications

1. Alliage à base de cuivre présentant une combinaison améliorée de limite d'élasticité, de 5conductivité électrique et de résistance à la relaxation de contrainte, composé de:
entre 3,5 et 3,9 pour cent en poids de Ni;
entre 0,8 et 1,0 pour cent en poids de Co;
entre 1,0 et 1,2 pour cent en poids de Si;
entre 0,05 et 0,15 pour cent en poids de Mg;
jusqu'à 0,1 pour cent en poids de Cr;
jusqu'à 1,0 pour cent en poids de Sn; et
jusqu'à 1,0 pour cent en poids de Mn,
le reste étant du cuivre et des impuretés,
dans lequel le rapport de Ni/Co est compris entre 3 et 5, l'alliage est traité de manière à présenter une limite d'élasticité d'au moins 140 ksi, et une conductivité électrique d'au moins 30 % IACS.

2. Alliage selon la revendication 1, dans lequel le rapport de (Ni+Co)/(Si-Cr/5) est compris entre 3,5 et 5,0.

3. Procédé de fabrication d'un alliage à base de cuivre selon l'une des revendications précédentes, comprenant les étapes suivantes:
faire fondre et couler l'alliage;
réaliser un laminage à chaud entre 750°C et 1050°C;
réaliser un laminage à froid à une épaisseur appropriée pour effectuer une mise en solution;
effectuer un recuit de mise en solution de l'alliage entre 800°C et 1050°C pendant 10 secondes à 1 heure; et
ensuite tremper ou refroidir rapidement l'alliage à la température ambiante afin d'obtenir une conductivité électrique inférieure à 20 % IACS (11,6 MS/m) et une taille de grain équiaxe de 5 µm à 20 µm;
laminer à froid l'alliage pour obtenir une réduction de l'épaisseur de 0 % à 75 %;
soumettre l'alliage à un recuit de durcissement à 300°C à 600°C pendant 10 minutes à 10 heures;
ensuite laminer à froid l'alliage pour obtenir une réduction de l'épaisseur de 10 % à 75 % jusqu'à l'épaisseur de finition; et
soumettre l'alliage à un second recuit de vieillissement à 250°C à 500°C pendant 10 minutes à 10 heures.

4. Procédé selon la revendication 3, comprenant en outre un recuit de recristallisation intermédiaire après le laminage à chaud.
